



US006153371A

# United States Patent [19]

Farid et al.

[11] Patent Number: 6,153,371

[45] Date of Patent: \*Nov. 28, 2000

[54] SILVER HALIDE LIGHT SENSITIVE EMULSION LAYER HAVING ENHANCED PHOTOGRAPHIC SENSITIVITY

[75] Inventors: **Samir Y. Farid**, Rochester; **Ian R. Gould**, Pittsford; **Stephen A. Godleski**, **Jerome R. Lenhard**, both of Fairport; **Annabel A. Muenter**; **Paul A. Zielinski**, both of Rochester, all of N.Y.

[73] Assignee: **Eastman Kodak Company**, Rochester, N.Y.

[\*] Notice: This patent is subject to a terminal disclaimer.

[21] Appl. No.: 09/118,552

[22] Filed: Jul. 17, 1998

## Related U.S. Application Data

[63] Continuation-in-part of application No. 08/900,694, Jul. 25, 1997, abandoned.

[51] Int. Cl.<sup>7</sup> G03C 1/10; G03C 1/12

[52] U.S. Cl. 430/581; 430/577; 430/578; 430/579; 430/580; 430/583; 430/584; 430/585; 430/586; 430/587; 430/590; 430/591; 430/592; 430/595; 430/600

[58] Field of Search 430/592, 581, 430/577, 578, 579, 580, 583, 584, 585, 586, 587, 590, 591, 594, 595, 600

## [56] References Cited

### U.S. PATENT DOCUMENTS

2,419,975 5/1947 Trivelli et al. .  
2,875,058 2/1959 Carroll et al. .  
2,937,089 5/1960 Jones et al. .  
3,457,078 7/1969 Riester .  
3,615,632 10/1971 Shiba et al. .  
3,695,888 10/1972 Hiller et al. .  
3,706,567 12/1972 Hiller et al. .  
3,809,561 7/1974 Ulbing et al. .  
4,607,006 8/1986 Hirano et al. .  
4,897,343 1/1990 Ikeda et al. .  
4,971,890 11/1990 Okada et al. .  
5,192,654 3/1993 Hioki et al. .  
5,306,612 4/1994 Philip et al. .  
5,436,121 7/1995 Suga et al. .  
5,459,052 10/1995 Skriver et al. .

5,478,719 12/1995 Hioki et al. .  
5,747,236 5/1998 Farid et al. ..... 430/583

### FOREIGN PATENT DOCUMENTS

474047 11/1992 European Pat. Off. .  
554856 A1 11/1993 European Pat. Off. .  
1064193 4/1967 United Kingdom .  
1255084 11/1971 United Kingdom .

### OTHER PUBLICATIONS

*The Theory of the Photographic Process*, Fourth Edition, T.H. James, Ed., pp. 265-266, (Macmillan, 1977).

Co-pending application Serial No. 08/740,536 (our docket No. 69500A) filed Oct. 30, 1997, entitled Silver Halide Light Sensitive Emulsion Layer Having Enhanced Photographic Sensitivity, Inventor(s) Farid et al.

Co-pending application Serial No. 08/739,911 (our docket No. 73257A) filed Oct. 30, 1996, entitled Silver Halide Light Sensitive Emulsion Layer Having Enhanced Photographic Sensitivity, Inventor(s) Farid et al.

Primary Examiner—Thorl Chea  
Attorney, Agent, or Firm—Edith A. Rice

## [57] ABSTRACT

This invention comprises a photographic element comprising a support and at least one silver halide emulsion layer in which the silver halide is sensitized with a compound of the formula:

Q-XY

wherein Q represents the atoms necessary to form a chromophore comprising an amidinium-ion, a carboxyl-ion or dipolar-amidic chromophoric system when conjugated with XY, and XY is a fragmentable electron donor moiety in which X is an electron donor group and Y is a leaving group other than hydrogen, and wherein:

- 1) XY has an oxidation potential between 0 and about 1.4 V;
- 2) the oxidized form of XY undergoes a bond cleavage reaction to give the radical X<sup>•</sup> and the leaving fragment Y.

In a preferred embodiment of the invention, the radical X<sup>•</sup> has an oxidation potential <-0.7V.

**31 Claims, No Drawings**

## SILVER HALIDE LIGHT SENSITIVE EMULSION LAYER HAVING ENHANCED PHOTOGRAPHIC SENSITIVITY

This application is a CIP of Ser. No. 08/900,694 filed Jul. 25, 1997 which is now abandoned.

### FIELD OF THE INVENTION

This invention relates to a photographic element comprising at least one light sensitive silver halide emulsion layer which has enhanced photographic sensitivity.

### BACKGROUND OF THE INVENTION

A variety of techniques have been used to improve the light-sensitivity of photographic silver halide materials.

Chemical sensitizing agents have been used to enhance the intrinsic sensitivity of silver halide. Conventional chemical sensitizing agents include various sulfur, gold, and group VIII metal compounds.

Spectral sensitizing agents, such as cyanine and other polymethine dyes, have been used alone, or in combination, to impart spectral sensitivity to emulsions in specific wavelength regions. These sensitizing dyes function by absorbing long wavelength light that is essentially unabsorbed by the silver halide emulsion and using the energy of that light to cause latent image formation in the silver halide.

Many attempts have been made to further increase the spectral sensitivity of silver halide materials. One method is to increase the amount of light captured by the spectral sensitizing agent by increasing the amount of spectral sensitizing agent added to the emulsion. However, a pronounced decrease in photographic sensitivity is obtained if more than an optimum amount of dye is added to the emulsion. This phenomenon is known as dye desensitization and involves sensitivity loss in both the spectral region wherein the sensitizing dye absorbs light, and in the light sensitive region intrinsic to silver halide. Dye desensitization has been described in *The Theory of the Photographic Process*, Fourth Edition, T. H. James, Editor, pages 265-266, (Macmillan, 1977).

It is also known that the spectral sensitivity found for certain sensitizing dyes can be dramatically enhanced by the combination with a second, usually colorless organic compound that itself displays no spectral sensitization effect. This is known as the supersensitizing effect.

Examples of compounds which are conventionally known to enhance spectral sensitivity include sulfonic acid derivatives (U.S. Pat. Nos. 2,937,089 and 3,706,567), triazine compounds described in U.S. Pat. Nos. 2,875,058 and 3,695,888, mercapto compounds described in U.S. Pat. No. 3,457,078, thiourea compounds described in U.S. Pat. No. 3,458,318, pyrimidine derivatives described in U.S. Pat. No. 3,615,632, dihydropyridine compounds described in U.S. Pat. No. 5,192,654, aminothiatriazoles as described in U.S. Pat. No. 5,306,612 and hydrazines as described in U.S. Pat. Nos. 2,419,975, 5,459,052 and 4,971,890 and European Patent Application No. 554,856 A1. The sensitivity increases obtained with these compounds generally are small, and many of these compounds have the disadvantage that they have the undesirable effect of deteriorating the stability of the emulsion or increasing fog.

Various electron donating compounds have also been used to improve spectral sensitivity of silver halide materials. U.S. Pat. No. 3,695,588 discloses that the electron donor ascorbic acid can be used in combination with a specific

tricarbocyanine dye to enhance sensitivity in the infrared region. The use of ascorbic acid to give spectral sensitivity improvement, when used in combination with specific cyanine and merocyanine dyes is also described in U.S. Pat. No.

5 3,809,561, British Patent No. 1,255,084, and British Patent No. 1,064,193. U.S. Pat. No. 4,897,343 discloses an improvement that decreases dye desensitization by the use of the combination of ascorbic acid, a metal sulfite compound, and a spectral sensitizing dye.

10 Electron-donating compounds that are covalently attached to a sensitizing dye or a silver-halide adsorptive group have also been used as supersensitizing agents. U.S. Pat. Nos. 5,436,121 and 5,478,719 disclose sensitivity improvements with the use of compounds containing electron-donating styryl bases attached to monomethine dyes. Spectral sensitivity improvements are also described in U.S. Pat. No. 4,607,006 for compounds containing an electron-donative group derived from a phenothiazine, phenoxazine, carbazole, dibenzophenothiazine, ferrocene, tris(2,2'-bipyridyl)ruthenium, or a triarylamine skeleton which are connected to a silver halide adsorptive group. However, most of these latter compounds have no silver halide sensitizing effect of their own and provide only minus-blue sensitivity improvements when used in combination with a sensitizing dye.

15 In commonly assigned, co-pending application Ser. No. 08/740,536 filed Oct. 30, 1996, the entire disclosures of which are incorporated herein by reference, that, when incorporated into a silver halide emulsion, provide a sensitizing effect alone or in combination with dyes. These compounds donate at least one electron and are fragmentable, i.e., they undergo a bond cleavage reaction other than deprotonation. In our commonly assigned, co-pending application Ser. No. 08/739,911 filed Oct. 30, 1996, the entire disclosures of which are incorporated herein by reference, we have disclosed the attachment of such fragmentable electron donors to sensitizing dyes. The attachment of the fragmentable electron donors to the sensitizing dyes is accomplished by a covalent bond comprising 20 an organic linking group that contains at least one C, N, S, or O atom.

### PROBLEM TO BE SOLVED BY THE INVENTION

25 There is a continuing need for materials which, when added to photographic emulsions, increase their sensitivity. Ideally such materials should be usable with a wide range of emulsion types, their activity should be controllable and they should not increase fog beyond acceptable limits. This invention provides such materials.

### SUMMARY OF THE INVENTION

30 As discussed above, commonly assigned, co-pending application Ser. No. 08/739,911 filed Oct. 30, 1996, the entire disclosures of which are incorporated herein by reference, discloses fragmentable electron donors that are attached to sensitizing dyes by a covalent bond comprising 35 an organic linking group that contains at least one C, N, S, or O atom. We have now discovered sensitizing dyes that contain a fragmentable electron donor moiety as an integral part of their chromophore structures.

40 We have now discovered that materials which improve sensitivity of photographic emulsions can be incorporated into the chromophore of a spectral sensitizing dye to provide the added advantage of increased emulsion efficiency at 45 relatively low concentrations.

In accordance with this invention, a silver halide emulsion layer of a photographic element is sensitized with a fragmentable electron donor moiety that upon donating an electron, undergoes a bond cleavage reaction other than deprotonation. The term "sensitization" is used in this patent application to mean an increase in the photographic response of the silver halide emulsion layer of a photographic element. The term "sensitizer" is used to mean a compound that provides sensitization when present in a silver halide emulsion layer.

One aspect of this invention comprises a photographic element comprising at least one silver halide emulsion layer in which the silver halide is sensitized with a compound of the formula:

Q-XY

wherein Q represents the atoms necessary to form a chromophore comprising an amidinium-ion, a carboxyl-ion or dipolar-amidic chromophoric system when conjugated with XY, and XY is a fragmentable electron donor moiety in which X is an electron donor group and Y is a leaving group other than hydrogen, and wherein:

1) XY has an oxidation potential between 0 and about 1.4 V; and

2) the oxidized form of XY undergoes a bond cleavage reaction to give the radical X<sup>•</sup> and the leaving fragment Y.

Another aspect of this invention comprises a photographic element comprising at least one silver halide emulsion layer in which the silver halide is sensitized with a compound of the formula:

Q-XY

wherein Q represents the atoms necessary to form a chromophore comprising an amidinium-ion, a carboxyl-ion or dipolar-amidic chromophoric system when conjugated with XY, and XY is a fragmentable electron donor moiety in which X is an electron donor group and Y is a leaving group other than hydrogen, and wherein:

1) XY has an oxidation potential between 0 and about 1.4 V;

2) the oxidized form of XY undergoes a bond cleavage reaction to give the radical X<sup>•</sup> and the leaving fragment Y; and

3) the radical X<sup>•</sup> has an oxidation potential  $\leq -0.7V$  (that is, equal to or more negative than about -0.7V).

Compounds which meet criteria (1) and (2) but not (3) are capable of donating one electron and are referred to herein as fragmentable one-electron donors. Compounds which meet all three criteria are capable of donating two electrons and are referred to herein as fragmentable two-electron donors.

In this patent application, oxidation potentials are reported as "V" which represents "volts versus a saturated calomel reference electrode".

#### ADVANTAGEOUS EFFECT OF THE INVENTION

This invention provides a silver halide photographic emulsion containing an organic electron donor capable of enhancing both the intrinsic and spectral sensitivity of the silver halide emulsion. The activity of these compounds can be easily varied with substituents to control their speed and fog effects in a manner appropriate to the particular silver halide emulsion in which they are used. An important feature

of these compounds is that they contain a sensitizing dye moiety, so as to minimize the amount of additive needed to produce a beneficial effect in the emulsion. These compounds may be used alone or in combination with other sensitizing dyes typically used to sensitize silver halide photographic emulsions.

Sensitizing dyes that contain the fragmentable electron donor moiety as part of its chromophore in accordance with this invention have an advantage in that they are easier to synthesize than sensitizing dyes wherein the electron donor is attached using distinct organic linking groups. The integration of the fragmentable electron donor moiety into the sensitizing dye chromophore should promote adhesion to the silver halide grain surface, thereby allowing the beneficial sensitizing effects at lower concentrations of the fragmentable electron donor. Because sensitizing dyes are required to be present to impart spectral sensitivity in specific spectral regions, use of a sensitizing dye with an incorporated fragmentable electron donating moiety allows the fragmentable electron donating compound to be close to the surface of the silver halide without displacing the primary spectral sensitizing agent.

#### DETAILED DESCRIPTION OF THE INVENTION

The photographic element of this invention comprises a silver halide emulsion layer which contains a fragmentable electron donating sensitizer molecule represented by the formula:

Q-XY

which when added to a silver halide emulsion, alone or in combination with a second spectral sensitizing dye, can increase the photographic sensitivity of the silver halide emulsion. The molecule Q-XY is comprised of two parts which when connected together form a chromophore comprising an amidinium-ion, a carboxyl-ion or dipolar-amidic chromophoric system that is generally found in cyanine, complex cyanine, hemicyanine, merocyanine, and complex merocyanine dyes as described in F. M. Hamer, *The Cyanine Dyes and Related Compounds* (Interscience Publishers, New York, 1964).

In a preferred embodiment of the invention, Q is represented by the general formulae VIII–XI below:



wherein:

E<sub>1</sub> represents the atoms necessary to form a substituted or unsubstituted hetero ring

each J independently represents a substituted or unsubstituted methine group,

q is a positive integer of from 1 to 4,

p represents 0 or 1,

D<sub>1</sub> represents a substituted or unsubstituted alkyl or substituted or unsubstituted aryl,

and,  $W_2$  is a counterion as necessary to balance the charge;



(IX)

wherein J and q are as defined above for formula (VIII) and G represents



wherein  $E_2$  represents the atoms necessary to complete a substituted or unsubstituted heterocyclic nucleus; and F and F' each independently represents a cyano group, an ester group, an acyl group, a carbamoyl group or an alkylsulfonyl group;

(X)



wherein  $D_1$ ,  $E_1$ , J, p, and q are as defined above for formula (IX); and  $E_3$  is defined the same as  $E_2$  for formula (IX) above;

(XI)



wherein  $E_3$ , J, G, and q, are as defined for formulae (IX) and (X) above;

In the above formulas,  $E_1$  represents the atoms necessary to complete a substituted or unsubstituted 5- or 6-membered heterocyclic nucleus which may include additional fused aromatic rings. These include a substituted or unsubstituted: thiazole nucleus, oxazole nucleus, selenazole nucleus, quinoline nucleus, tellurazole nucleus, pyridine nucleus, thiazoline nucleus, indoline nucleus, oxadiazole nucleus, thiadiazole nucleus, or imidazole nucleus. This nucleus may be substituted with known substituents, such as halogen (e.g., chloro, fluoro, bromo), alkoxy (e.g., methoxy, ethoxy), substituted or unsubstituted alkyl (e.g., methyl, trifluoromethyl), substituted or unsubstituted aryl, substituted or unsubstituted aralkyl, sulfonate, and others known in the art.

In one embodiment of the invention,  $E_1$  represents the atoms necessary to complete a substituted or unsubstituted thiazole nucleus, a substituted or unsubstituted selenazole nucleus, a substituted or unsubstituted imidazole nucleus, or a substituted or unsubstituted oxazole nucleus.

Examples of useful nuclei for  $E_1$  include: a thiazole nucleus, e.g., thiazole, 4-methylthiazole, 4-phenylthiazole, 5-methylthiazole, 5-phenylthiazole, 4,5-dimethyl-thiazole, 4,5-diphenylthiazole, 4-(2-thienyl)thiazole, benzothiazole, 4-chlorobenzothiazole, 5-chlorobenzothiazole, 6-chlorobenzothiazole, 7-chlorobenzothiazole,

- 4-methylbenzothiazole, 5-methylbenzothiazole, 6-methylbenzothiazole, 5-bromobenzothiazole, 6-bromobenzothiazole, 5-phenylbenzothiazole, 6-phenylbenzothiazole, 4-methoxybenzothiazole, 5-methoxybenzothiazole, 6-methoxybenzothiazole, 4-ethoxybenzothiazole, 5-ethoxybenzothiazole, tetrahydrobenzothiazole, 5,6-dimethoxybenzothiazole, 5,6-dioxymethylbenzothiazole, 5-hydroxybenzothiazole, 6,5-dihydroxybenzothiazole, naphtho[2,1-d]thiazole, 5-ethoxynaphtho[2,3-d]thiazole, 8-methoxynaphtho[2,3-d]thiazole, 7-methoxynaphtho[2,3-d]thiazole, 4'-methoxythianaphtho-7',6'-4,5-thiazole, etc.; an oxazole nucleus, e.g., 4-methyloxazole, 5-methyloxazole, 4-phenyloxazole, 4,5-diphenyloxazole, 4-ethyloxazole, 4,5-dimethyloxazole, 5-phenyloxazole, benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-ethoxybenzoxazole, 5-chlorobenzoxazole, 6-methoxybenzoxazole, 5-hydroxybenzoxazole, naphtho[2,1-d]oxazole, naphtho[1,2-d]oxazole, etc.; a selenazole nucleus, e.g., 4-methylselenazole, 4-phenylselenazole, benzoselenazole, 5-chlorobenzoselenazole, 5-methoxybenzoselenazole, 5-hydroxybenzoselenazole, tetrahydrobenzoselenazole, naphtho[2,1-d]selenazole, naphtho[1,2-d]selenazole, etc.; a pyridine nucleus, e.g., 2-pyridine, 5-methyl-2-pyridine, 4-pyridine, 3-methyl-4-pyridine, 3-methyl-4-pyridine, etc.; a quinoline nucleus, e.g., 2-quinoline, 3-methyl-2-quinoline, 5-ethyl-2-quinoline, 6-chloro-2-quinoline, 8-chloro-2-quinoline, 6-methoxy-2-quinoline, 8-ethoxy-2-quinoline, 8-hydroxy-2-quinoline, 4-quinoline, 6-methoxy-4-quinoline, 7-methyl-4-quinoline, 8-chloro-4-quinoline, etc.; a tellurazole nucleus, e.g., benzotellurazole, naphtho[1,2-d]benzotellurazole, 5,6-dimethoxybenzotellurazole, 5-methoxybenzotellurazole, 5-methylbenzotellurazole; a thiazoline nucleus, e.g., thiazoline, 4-methylthiazoline, etc.; a benzimidazole nucleus, e.g., benzimidazole, 5-trifluoromethylbenzimidazole, 5,6-dichlorobenzimidazole; and indole nucleus, 3,3-dimethylindole, 3,3-diethylindole, 3,3,5-trimethylindole; or a diazole nucleus, e.g., 5-phenyl-1,3,4-oxadiazole, 5-methyl-1,3,4-thiadiazole.
- Benzothiazole nuclei, naphthothiazole nuclei, benzoxazole nuclei, naphthoxazole nuclei, and benzimidazole nuclei are especially desirable.
- F and F' are each a cyano group, an ester group such as ethoxy carbonyl, methoxycarbonyl, etc., an acyl group, a carbamoyl group, or an alkylsulfonyl group such as ethylsulfonyl, methylsulfonyl, etc.
- $E_2$  represents the atoms necessary to complete a substituted or unsubstituted acidic heterocyclic nucleus, and these may take the form of any of the nuclei generally found in merocyanine dyes. Examples of useful nuclei for  $E_2$  include a 2-thio-2,4-oxazolidinedione nucleus (i.e., those of the 2-thio-2,4-(3H,5H)-oxaazolidinone series) (e.g., 3-ethyl-2-thio-2,4-oxazolidinedione, 3-(2-sulfoethyl)-2-thio-2,4-oxazolidinedione, 3-(4-sulfonylbutyl)-2-thio-2,4-oxazolidinedione, 3-(3-carboxypropyl)-2-thio-2,4-oxazolidinedione, etc.; a thianaphthoerone nucleus (e.g., 2-(2H)-thianaphthoerone, etc.), a 2-thio-2,5-thiazolidinedione nucleus (i.e., the 2-thio-2,5-(3H,4H)-thiazoledeione series) (e.g., 3-ethyl-2-thio-2,5-thiazolidinedione, etc.); a 2,4-thiazolidinedione nucleus (e.g., 2,4-thiazolidinedione, 3-ethyl-2,4-thiazolidinedione, 3-phenyl-2,4-thiazolidinedione, 3-a-naphthyl-2,4-thiazolidinedione, etc.); a thiazolidinone nucleus (e.g.,

4-thiazolidinone, 3-ethyl-4-thiazolidinone, 3-phenyl-4-thiazolidinone, 3-a-naphthyl-4-thiazolidinone, etc.); a 2-thiazolin-4-one series (e.g., 2-ethylmercapto-2-thiazolin-4-one, 2-alkylphenylamino-2-thiazolin-4-one, 2-diphenylamino-2-thiazolin-4-one, etc.) a 2-imino-4-oxazolidinone (i.e., pseudohydantoin) series (e.g., 2,4-imidazolidinedione (hydantoin) series (e.g., 2,4-imidazolidinedione, 3-ethyl-2,4-imidazolidinedione, 3-phenyl-2,4-imidazolidinedione, 3-a-naphthyl-2,4-imidazolidinedione, 1,3-diethyl-2,4-imidazolidinedione, 1-ethyl-3-phenyl-2,4-imidazolidinedione, 1-ethyl-2-a-naphthyl-2,4-imidazolidinedione, 1,3-diphenyl-2,4-imidazolidinedione, etc.); a 2-thio-2,4-imidazolidinedione (i.e., 2-thiohydantoin) nucleus (e.g., 2-thio-2,4-imidazolidinedione, 3-ethyl-2-thio-2,4-imidazolidinedione, 3-(2-carboxyethyl)-2-thio-2,4-imidazolidinedione, 3-phenyl-2-thio-2,4-imidazolidinedione, 1,3-diethyl-2-thio-2,4-imidazolidinedione, 1-ethyl-3-phenyl-2-thio-2,4-imidazolidinedione, 1-ethyl-3-naphthyl-2-thio-2,4-imidazolidinedione, 1,3-diphenyl-2-thio-2,4-imidazolidinedione, etc.), 2-imidazolin-5-one, rhodanine, iso-rhodanine, barbituric acid, 2-thiobarbituric acid, chroman-2,4-dione, pyrido[1,2-a]pyrimidin-1,3-dione nuclei.

The rhodanine nucleus, 3-alkylrhodanine nucleus, the 3-alkyl-2-thioxazolidin-2,4-dione nucleus, the 3-alkyl-2-thiohydantoin nucleus, the 3-alkyl-2-thio-oxazolin-2,4-dione nucleus, the iso-rhodanine nucleus, the barbituric acid nucleus, and the 2-thiobarbituric acid nucleus are especially preferred.

According to the formulas (VII)–(XI), each J represents a substituted or unsubstituted methine group. Examples of substituents for the methine groups include alkyl (preferably of from 1 to 6 carbon atoms, e.g., methyl, ethyl, etc.) and aryl (e.g., phenyl). Additionally, substituents on the methine groups may form bridged linkages.

W2 represents a counterion as necessary to balance the charge of the dye molecule. Such counterions include cations and anions for example sodium, potassium, triethylammonium, tetramethylguanidinium, diisopropylammonium and tetrabutylammonium, chloride, bromide, iodide, para-toluene sulfonate and the like. More than one counterion may be used to balance the charge as necessary

D1 is a substituted or unsubstituted aryl (preferably of 6 to 15 carbon atoms), or more preferably, substituted or unsubstituted alkyl (preferably of from 1 to 6 carbon atoms). Examples of aryl include phenyl, tolyl, p-chlorophenyl, and p-methoxyphenyl. Examples of alkyl include methyl, ethyl, propyl, isopropyl, butyl, hexyl, cyclohexyl, decyl, dodecyl, etc., and substituted alkyl groups (preferably a substituted lower alkyl containing from 1 to 6 carbon atoms), such as a hydroxyalkyl group, e.g., 2-hydroxyethyl, 4-hydroxybutyl, etc., a carboxyalkyl group, e.g., 2-carboxyethyl, 4-carboxybutyl, etc., a sulfoalkyl group, e.g., 2-sulfoethyl, 3-sulfobutyl, 4-sulfobutyl, etc., a sulfatoalkyl group, etc., an acyloxyalkyl group, e.g., 2-acetoxyethyl, 3-acetoxypropyl, 4-butyroxybutyl, etc., an alkoxy carbonylalkyl group, e.g., 2-methoxycarbonyl ethyl, 4-ethoxycarbonylbutyl, etc., or an aralkyl group, e.g., benzyl, phenethyl, etc., The alkyl or aryl group may be substituted by one or more of the substituents on the above-described substituted alkyl groups.

Illustrative Q groups include:



9

-continued



10

-continued



10

Particularly preferred are Q groups of the formula:



20 wherein:

X<sub>2</sub> is; O, S, N, or C(RS<sub>2</sub>)<sub>2</sub>, where R<sub>52</sub> is substituted or unsubstituted alkyl.

each R<sub>50</sub> is independently a hydrogen atom, a halogen atom, a substituted or unsubstituted alkyl group, or substituted or unsubstituted aryl group;

a is an integer of 1-4; and

R<sub>51</sub> is substituted or unsubstituted alkyl, or substituted or unsubstituted aryl.

XY is a fragmentable electron donor moiety wherein X is an electron donor group and Y is a leaving group. The preparation of compounds of the formula X-Y is disclosed in co-pending application Ser. No. 08/740,536 filed Oct. 30, 1996, the entire disclosure of which is incorporated herein by reference. The following represents the reactions believed to take place when the XY moiety undergoes oxidation and fragmentation to produce a radical X•, which in a preferred embodiment undergoes further oxidation.



45

(E<sub>ox1</sub>)YX

≤ 1.4 V

(E<sub>ox2</sub>)X<sup>•</sup>

≤ -0.7 V

50 The structural features of the moiety XY are defined by the characteristics of the two parts, namely the fragment X and the fragment Y. The structural features of the fragment X determines the oxidation potential of the XY moiety (E<sub>ox1</sub>) and that of the radical X<sup>•</sup>(E<sub>ox2</sub>), whereas both the X and Y fragments affect the fragmentation rate of the oxidized moiety XY<sup>•+</sup>.

Preferred X groups are of the general formula:



and

## 11

-continued



The symbol "R" (that is R without a subscript) is used in all structural formulae in this patent application to represent a hydrogen atom or an unsubstituted or substituted alkyl group.

In structure (I):

m: 0, 1;

Z: O, S, Se, Te;

Ar: aryl group (e.g., phenyl, naphthyl, phenanthryl, anthryl); or heterocyclic group (e.g., pyridine, indole, benzimidazole, thiazole, benzothiazole, thiadiazole, etc.);

R<sub>1</sub>: R, carboxyl, amide, sulfonamide, halogen, NR<sub>2</sub>, (OH)<sub>n</sub>, (OR)<sub>n</sub>, or (SR)<sub>n</sub> where R' is alkyl or substituted alkyl;

n: 1-3;

R<sub>2</sub>: R, Ar';

R<sub>3</sub>: R, Ar';

R<sub>2</sub> and R<sub>3</sub> together can form 5- to 8-membered ring;

R<sub>2</sub> and Ar: can be linked to form 5- to 8-membered ring;

R<sub>3</sub> and Ar: can be linked to form 5- to 8-membered ring;

Ar': aryl group such as phenyl, substituted phenyl, or heterocyclic group (e.g., pyridine, benzothiazole, etc.)

R: a hydrogen atom or an unsubstituted or substituted alkyl group.

In structure (II):

Ar: aryl group (e.g., phenyl, naphthyl, phenanthryl); or heterocyclic group (e.g., pyridine, benzothiazole, etc.);

R<sub>4</sub>: a substituent having a Hammett sigma value of -1 to +1, preferably -0.7 to +0.7, e.g., R, OR, SR, halogen, CHO, C(O)R, COOR, CONR<sub>2</sub>, SO<sub>3</sub>R, SO<sub>2</sub>NR<sub>2</sub>, SO<sub>2</sub>R, SOR, C(S)R, etc.;

R<sub>5</sub>: R, Ar'

R<sub>6</sub> and R<sub>7</sub>: R, Ar'

R<sub>5</sub> and Ar: can be linked to form 5- to 8-membered ring;

R<sub>6</sub> and Ar: can be linked to form 5- to 8-membered ring (in which case, R<sub>6</sub> can be a hetero atom);

R<sub>5</sub> and R<sub>6</sub>: can be linked to form 5- to 8-membered ring;

R<sub>6</sub> and R<sub>7</sub>: can be linked to form 5- to 8-membered ring;

Ar': aryl group such as phenyl, substituted phenyl, heterocyclic group

R: hydrogen atom or an unsubstituted or substituted alkyl group.

A discussion on Hammett sigma values can be found in C. Hansch and R. W. Taft *Chem. Rev.* Vol 91, (1991) p 165, the disclosure of which is incorporated herein by reference.

In structure (III):

W=O, S, Se;

Ar: aryl group (e.g., phenyl, naphthyl, phenanthryl, anthryl); or heterocyclic group (e.g., indole, benzimidazole, etc.).

## 12

R<sub>8</sub>: R, carboxyl, NR<sub>2</sub>, (OR)<sub>n</sub>, or (SR)<sub>n</sub> (n=1-3);

R<sub>9</sub> and R<sub>10</sub>: R, Ar';

Ar': aryl group such as phenyl, substituted phenyl, or heterocyclic group (e.g., pyridine, benzothiazole, etc.)

R<sub>9</sub> and Ar: can be linked to form 5- to 8-membered ring; R: a hydrogen atom or an unsubstituted or substituted alkyl group.

In structure (IV):

"ring" represents a substituted or unsubstituted 5-, 6- or 7-membered unsaturated ring, preferably a heterocyclic ring.

Since X is an electron donor group (i.e., an electron rich organic group), the substituents on the aromatic groups (Ar and/or Ar'), for any particular X group should be selected so that X remains electron rich. For example, if the aromatic group is highly electron rich, e.g. anthracene, electron withdrawing substituents can be used, providing the resulting XY moiety has an oxidation potential of 0 to about 1.4 V. Conversely, if the aromatic group is not electron rich, electron donating substituents should be selected.

When reference in this application is made to a substituent "group" this means that the substituent may itself be substituted or unsubstituted (for example "alkyl group" refers to a substituted or unsubstituted alkyl). Generally, unless otherwise specifically stated, substituents on any "groups" referenced herein or where something is stated to be possibly substituted, include the possibility of any groups, whether substituted or unsubstituted, which do not destroy properties necessary for the photographic utility. It will also be understood throughout this application that reference to a compound of a particular general formula includes those compounds of other more specific formula which specific formula falls within the general formula definition. Examples of substituents on any of the mentioned groups can include known substituents, such as: halogen, for example, chloro, fluoro, bromo, iodo; alkoxy, particularly those with 1 to 12 carbon atoms (for example, methoxy, ethoxy); substituted or unsubstituted alkyl, particularly lower alkyl (for example, methyl, trifluoromethyl); alkenyl or thioalkyl (for example, methylthio or ethylthio), particularly either of those with 1 to 12 carbon atoms; substituted and unsubstituted aryl, particularly those having from 6 to 20 carbon atoms (for example, phenyl); and substituted or unsubstituted heteroaryl, particularly those having a 5- or 6-membered ring containing 1 to 3 heteroatoms selected from N, O, or S (for example, pyridyl, thienyl, furyl, pyrrolyl); and others known in the art. Alkyl substituents preferably contain 1 to 12 carbon atoms and specifically include "lower alkyl", that is having from 1 to 6 carbon atoms, for example, methyl, ethyl, and the like. Further, with regard to any alkyl group, alkylene group or alkenyl group, it will be understood that these can be branched or unbranched and include ring structures.

The Q groups (VIII)-(XI) are attached to the X group of the XY moiety in a conjugated manner to form a chromophore comprising an amidinium-ion, a carboxyl-ion or dipolar-amidic chromophoric system. Accordingly, the groups (VIII)-(XI) may be attached to the nitrogen atom or to the aryl group of X in structures (I)-(III), to the N atom of X in structures (I) and (II), or to the ring in structure (IV). Examples of preferred X groups are given below. For simplicity and because of the multiple possible sites, the attachment of group (VIII)-(XI) is not specifically indicated in the structures. Specific structures for Q-XY compounds are provided hereinafter.

13

The following are illustrative examples of the group X of general structure I:



14

In the structures of this patent application a designation such as —OR(NR<sub>2</sub>) indicates that either —OR or —NR<sub>2</sub> can be present.

The following are illustrative examples of the group X of general structure II:



**15**

$Z_2 = S, O, Se, NR, CR_2, CR=CR$ ,  
 $R_{13} = \text{alkyl, substituted alkyl or aryl, and}$   
 $R_{14} = H, \text{alkyl, substituted alkyl or aryl.}$

The following are illustrative examples of the group X of the general structure III:



$n = 1-3$

The following are illustrative examples of the group X of the general structure IV:



$Z_3 = O, S, Se, NR$   
 $R_{15} = R, OR, NR_2$   
 $R_{16} = \text{alkyl, substituted alkyl}$

Preferred Y groups are:

(1)  $X'$ , where  $X'$  is an X group as defined in structures I-IV and may be the same as or different from the X group to which it is attached



where  $M = Si, Sn$  or  $Ge$ ; and  $R' = \text{alkyl or substituted alkyl}$

**16**

-continued



where  $Ar'' = \text{aryl or substituted aryl}$

10 In preferred embodiments of this invention Y is  $COO-$  or  $Si(R)_3$  or an X group. Particularly preferred Y groups are  $COO-$  or  $Si(R)_3$ .

Preferred XY moieties are derived from X-Y compounds of the formulae given below (for simplicity, and because of 15 the multiple possible sites, the attachment of the Q group not specified):



| 25 | Cpd. No. | R <sub>17</sub>               | R <sub>18</sub>  | R <sub>19</sub> |
|----|----------|-------------------------------|------------------|-----------------|
|    | 1        | CH <sub>3</sub>               | H                | H               |
|    | 2        | C <sub>2</sub> H <sub>5</sub> | OH               | H               |
|    | 3        | CH <sub>3</sub>               | OH               | H               |
|    | 4        | C <sub>2</sub> H <sub>5</sub> | OH               | CH <sub>3</sub> |
| 30 | 5        | CH <sub>3</sub>               | OH               | CH <sub>3</sub> |
|    | 6        | C <sub>2</sub> H <sub>5</sub> | OCH <sub>3</sub> | CH <sub>3</sub> |
|    | 7        | CH <sub>3</sub>               | OCH <sub>3</sub> | CH <sub>3</sub> |
|    | 8        | C <sub>2</sub> H <sub>5</sub> | OCH <sub>3</sub> | H               |



| 40 | Cpd. No. | R <sub>20</sub>                                                | R <sub>21</sub>  | R <sub>22</sub> | R <sub>23</sub>                    |
|----|----------|----------------------------------------------------------------|------------------|-----------------|------------------------------------|
|    | 9        | OCH <sub>2</sub> CO <sub>2</sub> -                             | H                | H               | H                                  |
|    | 10       | OCH <sub>3</sub>                                               | H                | H               | H                                  |
|    | 11       | CH <sub>3</sub>                                                | H                | H               | H                                  |
|    | 12       | Cl                                                             | H                | H               | H                                  |
|    | 13       | H                                                              | H                | H               | H                                  |
|    | 14       | H                                                              | H                | CH <sub>3</sub> | H                                  |
|    | 15       | OCH <sub>3</sub>                                               | H                | CH <sub>3</sub> | H                                  |
|    | 16       | CH(CH <sub>3</sub> )C <sub>2</sub> H <sub>5</sub>              | H                | CH <sub>3</sub> | H                                  |
|    | 17       | CHO                                                            | H                | CH <sub>3</sub> | H                                  |
|    | 18       | SO <sub>3</sub> -                                              | H                | CH <sub>3</sub> | H                                  |
|    | 19       | SO <sub>2</sub> N(C <sub>2</sub> H <sub>5</sub> ) <sub>2</sub> | H                | CH <sub>3</sub> | H                                  |
|    | 20       | CH <sub>3</sub>                                                | H                | CH <sub>3</sub> | H                                  |
|    | 21       | OCH <sub>3</sub>                                               | OCH <sub>3</sub> | H               | H                                  |
|    | 22       | H                                                              | H                | H               | OCH <sub>2</sub> CO <sub>2</sub> - |



| 60 | Cpd. No. | R <sub>20</sub>   | R <sub>22</sub> | R <sub>24</sub> | R <sub>21</sub> |
|----|----------|-------------------|-----------------|-----------------|-----------------|
|    | 23       | OCH <sub>3</sub>  | CH <sub>3</sub> | H               | H               |
|    | 24       | H                 | CH <sub>3</sub> | H               | H               |
|    | 25       | CO <sub>2</sub> - | CH <sub>3</sub> | H               | H               |
|    | 26       | Cl                | CH <sub>3</sub> | H               | H               |
|    | 27       | CONH <sub>2</sub> | CH <sub>3</sub> | H               | H               |

-continued

|         |                                               |                                   |                                                 |                   |    |
|---------|-----------------------------------------------|-----------------------------------|-------------------------------------------------|-------------------|----|
| 28      | CO <sub>2</sub> C <sub>2</sub> H <sub>5</sub> | CH <sub>3</sub>                   | H                                               | H                 |    |
| 29      | CH <sub>3</sub>                               | CH <sub>2</sub> CO <sub>2</sub> — | H                                               | H                 |    |
| 30      | H                                             | CH <sub>2</sub> CO <sub>2</sub> — | H                                               | H                 |    |
| 31      | CO <sub>2</sub> —                             | CH <sub>2</sub> CO <sub>2</sub> — | H                                               | H                 |    |
| 32      | H                                             | CH <sub>3</sub>                   | H                                               | CONH <sub>2</sub> |    |
| 33      | CO <sub>2</sub> —                             | CH <sub>3</sub>                   | CH <sub>3</sub>                                 | H                 |    |
| 34      | H                                             | CH <sub>3</sub>                   | C <sub>2</sub> H <sub>5</sub>                   | CONH <sub>2</sub> |    |
| 35      | CH <sub>3</sub>                               | CH <sub>3</sub>                   | (CH <sub>2</sub> ) <sub>3</sub> CH <sub>3</sub> | H                 |    |
| 36      | OCH <sub>3</sub>                              | CH <sub>3</sub>                   | (CH <sub>2</sub> ) <sub>3</sub> CH <sub>3</sub> | H                 | 10 |
| 37      | H                                             | CH <sub>3</sub>                   | (CH <sub>2</sub> ) <sub>3</sub> CH <sub>3</sub> | H                 |    |
| 38      | CO <sub>2</sub> —                             | CH <sub>3</sub>                   | (CH <sub>2</sub> ) <sub>3</sub> CH <sub>3</sub> | H                 |    |
| 39      | Cl                                            | CH <sub>3</sub>                   | (CH <sub>2</sub> ) <sub>3</sub> CH <sub>3</sub> | H                 |    |
| 40      | CH <sub>3</sub>                               | CH <sub>2</sub> CO <sub>2</sub> — | (CH <sub>2</sub> ) <sub>3</sub> CH <sub>3</sub> | H                 |    |
| 41      | H                                             | CH <sub>2</sub> CO <sub>2</sub> — | (CH <sub>2</sub> ) <sub>3</sub> CH <sub>3</sub> | H                 |    |
| Cpd. 42 |                                               |                                   |                                                 |                   |    |
| Cpd. 43 |                                               |                                   |                                                 |                   |    |
| Cpd. 44 |                                               |                                   |                                                 |                   |    |
| Cpd. 45 |                                               |                                   |                                                 |                   |    |
| Cpd. 46 |                                               |                                   |                                                 |                   |    |
| Cpd. 47 |                                               |                                   |                                                 |                   |    |

-continued

|    |         |  |
|----|---------|--|
| 5  | Cpd. 48 |  |
| 10 | Cpd. 49 |  |
| 15 |         |  |
| 20 | Cpd. 50 |  |
| 25 | Cpd. 51 |  |
| 30 | Cpd. 52 |  |
| 35 |         |  |
| 40 | Cpd. 53 |  |
| 45 | Cpd. 54 |  |
| 50 |         |  |
| 55 | Cpd. 55 |  |
| 60 | Cpd. 56 |  |
| 65 |         |  |

-continued

Cpd. 57



Cpd. 58



Cpd. 59



Cpd. 60



Cpd. 61



Cpd. 62



Cpd. 63



Cpd. 64



Fragmentable electron donating moieties XY are derived from electron donating compounds X-Y which can be fragmentable one electron donating compounds which meet the first two criteria set forth below or fragmentable two electron donating compounds which meet all three criteria set forth below. The first criterion relates to the oxidation potential of X-Y ( $E_1$ ).  $E_1$  is preferably no higher than about 1.4 V and preferably less than about 1.0 V. The oxidation potential is preferably greater than 0, more preferably greater than about 0.3 V.  $E_1$  is preferably in the range of about 0 to about 1.4 V, and more preferably of from about 0.3 V to about 1.0 V.

Oxidation potentials are well known and can be found, for example, in "Encyclopedia of Electrochemistry of the Elements", Organic Section, Volumes XI-XV, A. Bard and H. Lund (Editors) Marcel Dekker Inc., NY (1984).  $E_1$  can be measured by the technique of cyclic voltammetry. In this technique, the electron donating compound is dissolved in a solution of 80%/20% by volume acetonitrile to water containing 0.1 M lithium perchlorate. Oxygen is removed from the solution by passing nitrogen gas through the solution for 10 minutes prior to measurement. A glassy carbon disk is used for the working electrode, a platinum wire is used for the counter electrode, and a saturated calomel electrode (SCE) is used for the reference electrode. Measurement is conducted at 25° C. using a potential sweep rate of 0.1 V/sec. The oxidation potential vs. SCE is taken as the peak potential of the cyclic voltammetric wave.  $E_1$  values for typical X-Y compounds useful in preparing the compounds of this invention are given in Table A.

TABLE A

| 40 | Compound | Oxidation Potential of X-Y |          |
|----|----------|----------------------------|----------|
|    |          | $E_1$ (V vs SCE)           | Compound |
|    | 1        | 0.53                       | 30       |
|    | 2        | 0.50                       | 26       |
|    | 5        | 0.51                       | 27       |
|    | 4        | 0.49                       | 38       |
|    | 7        | 0.52                       | 39       |
|    | 6        | 0.51                       | 41       |
|    | 8        | 0.49                       | 34       |
|    | 48       | 0.70                       | 28       |
|    | 51       | 0.91                       | 17       |
|    | 49       | ~1.2                       | 18       |
|    | 50       | ~1.05                      | 19       |
|    | 43       | 0.61                       | 31       |
|    | 44       | 0.64                       | 22       |
|    | 45       | 0.64                       | 59       |
|    | 46       | 0.68                       | 56       |
|    | 42       | 0.30                       | 57       |
|    | 9        | 0.38                       | 58       |
|    | 10       | 0.38                       | 52       |
|    | 11       | 0.46                       | 54       |
|    | 23       | 0.37                       |          |
|    | 20       | 0.46                       |          |
|    | 14       | 0.50                       |          |
|    | 15       | 0.36                       |          |
|    | 16       | 0.47                       |          |
|    | 36       | 0.22                       |          |
|    | 29       | 0.52                       |          |
|    | 40       | 0.38                       |          |
|    | 35       | 0.34                       |          |
|    | 25       | 0.62                       |          |
|    | 33       | 0.54                       |          |
|    | 13       | 0.54                       |          |

In the above formulae, counterion(s) required to balance the charge of the, XY moiety are not shown as any counterion can be utilized. Common counterions are sodium, potassium, triethylammonium (TEA<sup>+</sup>), tetramethylguanidinium (TMG<sup>+</sup>), diisopropylammonium (DIPA<sup>+</sup>), and tetrabutylammonium (TBA<sup>+</sup>).

TABLE A-continued

| Oxidation Potential of X-Y |                  |          |                  |
|----------------------------|------------------|----------|------------------|
| Compound                   | $E_1$ (V vs SCE) | Compound | $E_1$ (V vs SCE) |
| 12                         | 0.58             |          |                  |
| 21                         | 0.36             |          |                  |
| 24                         | 0.52             |          |                  |
| 37                         | 0.43             |          |                  |
| 32                         | 0.58             |          |                  |
| 60                         | 0.80             |          |                  |

The second criterion defining the fragmentable XY groups is the requirement that the oxidized form of X-Y, that is the radical cation X-Y<sup>+</sup>, undergoes a bond cleavage reaction to give the radical X<sup>·</sup> and the fragment Y<sup>+</sup> (or in the case of an anionic compound the radical X<sup>·</sup> and the fragment Y). This bond cleavage reaction is also referred to herein as "fragmentation". It is widely known that radical species, and in particular radical cations, formed by a one-electron oxidation reaction may undergo a multitude of reactions, some of which are dependent upon their concentration and on the specific environment wherein they are produced. As described in "Kinetics and Mechanisms of Reactions of Organic Cation Radicals in Solution", Advances in Physical Organic Chemistry, vol 20, 1984, pp 55-180, and "Formation, Properties and Reactions of Cation Radicals in Solution", Advances in Physical Organic Chemistry, vol 13, 1976, pp 156-264, V. Gold Editor, 1984, published by Academic Press, NY, the range of reactions available to such radical species includes: dimerization, deprotonation, hydrolysis, nucleophilic substitution, disproportionation, and bond cleavage. With compounds useful in accordance with our invention, the radical formed on oxidation of X-Y undergoes a bond cleavage reaction.

The kinetics of the bond cleavage or fragmentation reaction can be measured by conventional laser flash photolysis. The general technique of laser flash photolysis as a method to study properties of transient species is well known (see, for example, "Absorption Spectroscopy of Transient Species". Herkstroeter and I. R. Gould in Physical Methods of Chemistry Series, second Edition, Volume 8, page 225, edited by B. Rossiter and R. Baetzold, John Wiley & Sons, New York, 1993). The specific experimental apparatus we used to measure fragmentation rate constants and radical oxidation potentials is described in detail below. The rate constant of fragmentation in compounds useful in accordance with this invention is preferably faster than about 0.1 per second (i.e., 0.1 s<sup>-1</sup> or faster, or, in other words, the lifetime of the radical cation X-Y<sup>+</sup> should be 10 sec or less). The fragmentation rate constants can be considerably higher than this, namely in the 10<sup>2</sup> to 10<sup>13</sup> s<sup>-1</sup> range. The fragmentation rate constant is preferably about 0.1 sec<sup>-1</sup> to about 10<sup>13</sup> s<sup>-1</sup>, more preferably about 10<sup>2</sup> to about 10<sup>9</sup> s<sup>-1</sup>. Fragmentation rate constants  $k_f$ (s<sup>-1</sup>) for typical compounds useful in preparing the compounds of this invention are given in Table B.

TABLE B

| Rate Constants for Decarboxylation of Radical Cations in CH <sub>3</sub> CN/H <sub>2</sub> O (4:1) |                          |                 |                                              |                                              |                          |  |  |  |
|----------------------------------------------------------------------------------------------------|--------------------------|-----------------|----------------------------------------------|----------------------------------------------|--------------------------|--|--|--|
| COMP'D                                                                                             | R <sub>26</sub>          | R <sub>27</sub> | R <sub>28</sub>                              | R <sub>29</sub>                              | $k_f$ (s <sup>-1</sup> ) |  |  |  |
| 14                                                                                                 | H                        | H               | Me                                           | CH <sub>2</sub> CO <sub>2</sub> <sup>·</sup> | >2.0 × 10 <sup>7</sup>   |  |  |  |
| 13                                                                                                 | H                        | H               | H                                            | CH <sub>2</sub> CO <sub>2</sub> <sup>·</sup> | 1.7 × 10 <sup>7</sup>    |  |  |  |
| 20                                                                                                 | Me                       | H               | Me                                           | CH <sub>2</sub> CO <sub>2</sub> <sup>·</sup> | 8.1 × 10 <sup>6</sup>    |  |  |  |
| 11                                                                                                 | Me                       | H               | H                                            | CH <sub>2</sub> CO <sub>2</sub> <sup>·</sup> | 1.6 × 10 <sup>6</sup>    |  |  |  |
| 15                                                                                                 | OMe                      | H               | Me                                           | CH <sub>2</sub> CO <sub>2</sub> <sup>·</sup> | 9.0 × 10 <sup>4</sup>    |  |  |  |
| 10                                                                                                 | OMe                      | H               | H                                            | CH <sub>2</sub> CO <sub>2</sub> <sup>·</sup> | 9.3 × 10 <sup>3</sup>    |  |  |  |
| 21                                                                                                 | OMe                      | OMe             | H                                            | CH <sub>2</sub> CO <sub>2</sub> <sup>·</sup> | 1 × 10 <sup>3</sup>      |  |  |  |
| 36                                                                                                 | OMe                      | H               | Me                                           | n-Bu                                         | 1.1 × 10 <sup>6</sup>    |  |  |  |
| 40                                                                                                 | Me                       | H               | CH <sub>2</sub> CO <sub>2</sub> <sup>·</sup> | n-Bu                                         | 1.3 × 10 <sup>7</sup>    |  |  |  |
| 29                                                                                                 | Me                       | H               | CH <sub>2</sub> CO <sub>2</sub> <sup>·</sup> | H                                            | 5.4 × 10 <sup>6</sup>    |  |  |  |
| 54                                                                                                 | Me                       | H               | Me                                           | H                                            | 1.4 × 10 <sup>7</sup>    |  |  |  |
| COMPOUND                                                                                           | R <sub>30</sub>          | R <sub>31</sub> | $k_f$ (s <sup>-1</sup> )                     |                                              |                          |  |  |  |
| 3                                                                                                  | OH                       | Me              | 5.5 × 10 <sup>5</sup>                        |                                              |                          |  |  |  |
| 1                                                                                                  | H                        | H               | ~3.0 × 10 <sup>5</sup>                       |                                              |                          |  |  |  |
| COMPOUND                                                                                           | $k_f$ (s <sup>-1</sup> ) |                 |                                              |                                              |                          |  |  |  |
| 47                                                                                                 | >10 <sup>7</sup>         |                 |                                              |                                              |                          |  |  |  |
| COMPOUND                                                                                           | $k_f$ (s <sup>-1</sup> ) |                 |                                              |                                              |                          |  |  |  |
| 52                                                                                                 | >10 <sup>9</sup>         |                 |                                              |                                              |                          |  |  |  |
| 53                                                                                                 | >10 <sup>9</sup>         |                 |                                              |                                              |                          |  |  |  |
| COMPOUND                                                                                           | $k_f$ (s <sup>-1</sup> ) |                 |                                              |                                              |                          |  |  |  |
| 55                                                                                                 | >10 <sup>9</sup>         |                 |                                              |                                              |                          |  |  |  |
| COMPOUND                                                                                           | $k_f$ (s <sup>-1</sup> ) |                 |                                              |                                              |                          |  |  |  |
| 60                                                                                                 | >10 <sup>9</sup>         |                 |                                              |                                              |                          |  |  |  |
| COMPOUND                                                                                           | $k_f$ (s <sup>-1</sup> ) |                 |                                              |                                              |                          |  |  |  |
| 65                                                                                                 | >10 <sup>9</sup>         |                 |                                              |                                              |                          |  |  |  |

TABLE B-continued

| Rate Constants for Decarboxylation of Radical Cations in $\text{CH}_3\text{CN}/\text{H}_2\text{O}$ (4:1) |                                 |
|----------------------------------------------------------------------------------------------------------|---------------------------------|
| 44                                                                                                       | $5.3 \times 10^5$               |
| 5                                                                                                        |                                 |
| COMPOUND                                                                                                 | $k_{\text{fr}} (\text{s}^{-1})$ |
| 56                                                                                                       | $1.2 \times 10^5$               |
|                                                                                                          |                                 |
| 20                                                                                                       |                                 |
| COMPOUND                                                                                                 | $k_{\text{fr}} (\text{s}^{-1})$ |
| 57                                                                                                       | ca. $1 \times 10^5$             |
| 25                                                                                                       |                                 |

In a preferred embodiment of the invention, the XY moiety is a fragmentable two-electron donor moiety and meets a third criterion, that the radical X<sup>•</sup> resulting from the bond cleavage reaction has an oxidation potential equal to or more negative than -0.7 V, preferably more negative than about -0.9 V. This oxidation potential is preferably in the range of from about -0.7 to about -2 V, more preferably from about -0.8 to about -2 V and most preferably from about -0.9 to about -1.6 V.

The oxidation potential of many radicals have been measured by transient electrochemical and pulse radiolysis techniques as reported by Wayner, D. D.; McPhee, D. J.; Griller, D. in *J Am. Chem. Soc.* 1988, 110, 132; Rao, P. S.; Hayon, E. *J. Am. Chem. Soc.* 1974, 96, 1287 and Rao, P. S.; Hayon, E. *J. Am. Chem. Soc.* 1974, 96, 1295. The data demonstrate that the oxidation potentials of tertiary radicals are less positive (i.e., the radicals are stronger reducing agents) than those of the corresponding secondary radicals, which in turn are more negative than those of the corresponding primary radicals. For example, the oxidation potential of benzyl radical decreases from 0.73 V to 0.37 V to 0.16 V upon replacement of one or both hydrogen atoms by methyl groups.



A considerable decrease in the oxidation potential of the radicals is achieved by a hydroxy or alkoxy substituents. For example the oxidation potential of the benzyl radical (+0.73 V) decreases to -0.44 when one of the hydrogen atoms is replaced by a methoxy group.



An  $\alpha$ -amino substituent decreases the oxidation potential of the radical to values of about -1 V.

In accordance with our invention we have discovered that compounds which provide a radical X<sup>•</sup> having an oxidation potential more negative than -0.7 are particularly advantageous for use in sensitizing silver halide emulsions. As set forth in the above-noted articles, the substitution at the  $\alpha$  carbon atom influences the oxidation potential of the radical. We have found that substitution of the phenyl moiety with at least one electron donating substituent or replacement of the phenyl with an electron donating aryl or heterocyclic group also influences the oxidation potential of X<sup>•</sup>. Illustrative examples of X<sup>•</sup> having an oxidation potential more negative than -0.7 are given below in Table C. The oxidation potential of the transient species X<sup>•</sup>, can be determined using a laser flash photolysis technique as described in greater detail below.

In this technique, the compound X-Y is oxidized by an electron transfer reaction initiated by a short laser pulse. The oxidized form of X-Y then undergoes the bond cleavage reaction to give the radical X<sup>•</sup>. X<sup>•</sup> is then allowed to interact with various electron acceptor compounds of known reduction potential. The ability of X<sup>•</sup> to reduce a given electron acceptor compound indicates that the oxidation potential of X<sup>•</sup> is nearly equal to or more negative than the reduction potential of that electron acceptor compound. The experimental details are set forth more fully below. The oxidation potentials (E<sub>2</sub>) for radicals X<sup>•</sup> for typical compounds useful in accordance with our invention are given in Table C. Where only limits on potentials could be determined, the following notation is used: <-0.90 V should be read as "more negative than -0.90 V" and >0.40 V should be read as "less negative than -0.40 V".

Illustrative X<sup>•</sup> radicals useful in accordance with the third criterion of our invention are those given below having an oxidation potential E<sub>2</sub> more negative than -0.7 V. Some comparative examples with E<sub>2</sub> less negative than -0.7 V are also included.

TABLE C

| Oxidation Potentials of Radicals (X <sup>•</sup> ), E <sub>2</sub> |                 |                 |                |
|--------------------------------------------------------------------|-----------------|-----------------|----------------|
| Parent X-Y compound                                                | R <sub>33</sub> | R <sub>34</sub> | E <sub>2</sub> |
| 46                                                                 | H               | H               | ~-0.34         |
| 45                                                                 | Me              | H               | -0.56          |
| 44                                                                 | Me              | Me              | -0.81          |
| 65                                                                 | OH              | H               | -0.89          |
| 43                                                                 |                 |                 |                |

TABLE C-continued

| Oxidation Potentials of Radicals (X <sup>•</sup> ), E <sub>2</sub> |                              |                 |                 |        |
|--------------------------------------------------------------------|------------------------------|-----------------|-----------------|--------|
| Parent X-Y compound                                                | R <sub>35</sub>              | R <sub>36</sub> | E <sub>2</sub>  |        |
| 13                                                                 | H                            | H               | ~-0.85          |        |
| 14                                                                 | H                            | Me              | <-0.9           |        |
| 11                                                                 | Me                           | H               | ~-0.9           |        |
| 16                                                                 | i-Bu                         | H               | ~-0.9           |        |
| 20                                                                 | Me                           | Me              | <-0.9           |        |
| 10                                                                 | OMe                          | H               | ~-0.9           |        |
| 15                                                                 | OMe                          | Me              | <-0.9           |        |
|                                                                    |                              |                 |                 |        |
|                                                                    |                              |                 |                 |        |
| Parent X-Y compound                                                | R <sub>37</sub>              | R <sub>38</sub> | R <sub>39</sub> |        |
| 8                                                                  | Et                           | H               | OMe             | ~-0.85 |
| 2                                                                  | Et                           | H               | OH              | <-0.9  |
| 7                                                                  | Me                           | Me              | OMe             | <-0.9  |
| 5                                                                  | Me                           | Me              | OH              | <-0.9  |
| 1                                                                  | Me                           | H               | H               | >-0.5  |
|                                                                    |                              |                 |                 |        |
|                                                                    |                              |                 |                 |        |
| Parent X-Y compound                                                | R <sub>40</sub>              | R <sub>41</sub> | R <sub>42</sub> |        |
| 36                                                                 | OMe                          | Me              | n-Bu            | <-0.9  |
| 33                                                                 | CO <sub>2</sub> <sup>-</sup> | Me              | Me              | <-0.9  |
|                                                                    |                              |                 |                 |        |
|                                                                    |                              |                 |                 |        |
| Parent X-Y compound                                                | R <sub>44</sub>              | R <sub>43</sub> | R <sub>46</sub> |        |
| 48                                                                 | OMe                          | OMe             | OMe             | <-0.9  |
| 51                                                                 | OMe                          | H               | OMe             | <-0.9  |
| 49                                                                 | H                            | H               | H               | -0.75  |
| 50                                                                 | OMe                          | H               | H               | <-0.9  |
|                                                                    |                              |                 |                 |        |
|                                                                    |                              |                 |                 |        |
| Parent X-Y compound                                                | R <sub>44</sub>              | R <sub>43</sub> | R <sub>46</sub> |        |
| 42                                                                 | ~-0.9                        |                 |                 |        |

TABLE C-continued

| Oxidation Potentials of Radicals (X <sup>•</sup> ), E <sub>2</sub> |                 |                |  |
|--------------------------------------------------------------------|-----------------|----------------|--|
| Parent X-Y compound                                                | R <sub>32</sub> | E <sub>2</sub> |  |
| 47                                                                 |                 | <-0.9          |  |
|                                                                    |                 |                |  |
|                                                                    |                 |                |  |
| Parent X-Y compound                                                | R <sub>32</sub> | E <sub>2</sub> |  |
| 52                                                                 | H               | <-0.9          |  |
| 53                                                                 | Et              | <-0.9          |  |
|                                                                    |                 |                |  |
|                                                                    |                 |                |  |
| Parent X-Y compound                                                | R <sub>32</sub> | E <sub>2</sub> |  |
| 54                                                                 |                 | <-0.9          |  |
|                                                                    |                 |                |  |
|                                                                    |                 |                |  |
| Parent X-Y compound                                                | R <sub>32</sub> | E <sub>2</sub> |  |
| 29                                                                 |                 | <-0.9          |  |
|                                                                    |                 |                |  |
|                                                                    |                 |                |  |
| Parent X-Y compound                                                | R <sub>32</sub> | E <sub>2</sub> |  |
| 56                                                                 |                 | <-0.9          |  |
|                                                                    |                 |                |  |

TABLE C-continued

| Oxidation Potentials of Radicals (X <sup>•</sup> ), E <sub>2</sub> |                |
|--------------------------------------------------------------------|----------------|
| Parent X-Y compound                                                | E <sub>2</sub> |



TABLE C-continued

| Oxidation Potentials of Radicals (X <sup>•</sup> ), E <sub>2</sub> |
|--------------------------------------------------------------------|
| 5<br>57<br><0.9                                                    |

10 Specific inventive compounds according to the general formulae given above are listed below, but the present invention should not be construed as being limited thereto. As is demonstrated in these examples, the point of attachment of Q to XY may be at one of the heteroatoms or at one of the aromatic or heterocyclic rings on the X portion of XY.



-continued

INV 12

INV 13



INV 14



INV 15



INV 16



INV 17

INV 18



INV 19

INV 20



INV 21





INV 23

INV 24



INV 25

INV 26



INV 27

INV 28



INV 29

INV 30





-continued

INV 40



INV 41



INV 42



INV 43



INV 44



INV 45



In the above formulae, counterion(s) required to balance the net charge of a Q-XY compound are not shown as any counterion can be utilized. Common counterions that can be used include sodium, potassium, triethylammonium (TEA<sup>+</sup>), tetramethylguanidinium (TMG<sup>+</sup>), diisopropylammonium (DIPA<sup>+</sup>), and tetrabutylammonium (TBA<sup>+</sup>).

Table D combines electrochemical and laser flash photolysis data for the XY moiety contained in selected fragmentable electron donating sensitizers according to the formula Q-XY. Specifically, this Table contains data for E<sub>1</sub>, the oxidation potential of the parent fragmentable electron donating moiety X-Y; k<sub>f</sub>, the fragmentation rate of the

55 oxidized X-Y (including X-Y<sup>+</sup>); and E<sub>2</sub>, the oxidation potential of the radical X<sup>•</sup>. In Table D, these characteristic properties of the moiety XY are reported for the model compound where Q has been replaced by a formyl group in INV 2, and INV 10, or by hydrogen or alkyl in INV 20 and INV 27. In the actual compounds Q-XY, these characteristic properties may vary slightly from the values for the model compounds but will not be greatly perturbed. The data in Table D illustrate Q-XY compounds useful in this invention that are fragmentable two-electron donating sensitizers and meet all the three criteria set forth above.

TABLE D

| Compound | $E_1$ (V)<br>for XY moiety | $k_{f1}$ (s <sup>-1</sup> )<br>for XY moiety | $E_2$ (V)<br>for XY moiety |
|----------|----------------------------|----------------------------------------------|----------------------------|
| Inv 2    | 0.74                       | >10 <sup>7</sup>                             | <-0.9                      |
| Inv 6    | 0.69                       | >10 <sup>7</sup>                             | <-0.75                     |
| Inv 10   | 0.74                       | 1.7 × 10 <sup>11</sup>                       | <-0.9                      |
| Inv 20   | 0.49                       | >10 <sup>7</sup>                             | <-0.9                      |
| Inv 27   | 0.64                       | 5.3 × 10 <sup>5</sup>                        | -0.81                      |

-continued

COMP 6



COMP 7



COMP 8



COMP 9



COMP 10



COMP 11



COMP 1



COMP 2



COMP 3



COMP 4



COMP 5

In the above formulae, counterion(s) required to balance the net charge of a Q-XY compound are not shown as any counterion can be utilized. Common cationic counterions that can be used include sodium, potassium, triethylammonium (TEA<sup>+</sup>), tetramethylguanidinium (TMG<sup>+</sup>), diisopropylammonium (DIPA<sup>+</sup>), and tetrabutylammonium (TBA<sup>+</sup>). Common anionic counterions include halogen ions (e.g., chlorine, bromide, iodide, etc.), p-toluenesulfonate, p-chlorobenzene sulfonate, methane sulfonate, tetrafluoroborate ion, perchlorate ion, methylsulfate ion and ethylsulfate ion.

The fragmentable electron donors useful in this invention are vastly different from the silver halide adsorptive (one)-electron donors described in U.S. Pat. No. 4,607,006. The electron donating moieties described therein, for example phenothiazine, phenoxazine, carbazole, dibenzophenothiazine, ferrocene, tris(2,2'-bipyridyl) ruthenium, or a triarylamine, are well known for forming extremely stable, i.e., non-fragmentable, radical cations as noted in the following references J. Heterocyclic Chem., vol. 12, 1975, pp 397-399, J. Org. Chem., vol 42, 1977, pp 983-988, "The Encyclopedia of Electrochemistry of the Elements", Vol XIII, pp 25-33, A. J. Bard Editor, published by Marcel Dekker Inc., Advances in Physical organic Chemistry, vol 20, pp 55-180, V. Gold Editor, 1984, published by Academic Press, NY. Also, the electron donating adsorptive compounds of U.S. Pat. No. 4,607,006 donate only one electron per molecule upon oxidation. In a preferred embodiment of the present invention, the fragmentable electron donors are capable of donating two electrons.

These fragmentable electron donors of the present invention also differ from other known photographically active

compounds such as R-typing agents, nucleators, and stabilizers. Known R-typing agents, such as Sn complexes, thiourea dioxide, borohydride, ascorbic acid, and amine boranes are very strong reducing agents. These agents typically undergo multi-electron oxidations but have oxidation potentials more negative than 0 V vs SCE. For example the oxidation potential for  $\text{SnCl}_2$  is reported in CRC Handbook of Chemistry and Physics, 55th edition, CRC Press Inc., Cleveland, Ohio 1975, pp D122 to be  $\sim -0.10$  V and that for borohydride is reported in J. Electrochem. Soc., 1992, vol. 139, pp 2212-2217 to be  $-0.48$  V vs SCE. These redox characteristics allow for an uncontrolled reduction of silver halide when added to silver halide emulsions, and thus the obtained sensitivity improvements are very often accompanied by undesirable levels of fog. Conventional nucleator compounds such as hydrazines and hydrazides differ from the fragmentable electron donors described herein in that nucleators are usually added to photographic emulsions in an inactive form. Nucleators are transformed into photographically active compounds only when activated in a strongly basic solution, such as a developer solution, wherein the nucleator compound undergoes a deprotonation or hydrolysis reaction to afford a strong reducing agent. In further contrast to the fragmentable electron donors, the oxidation of traditional R-typing agents and nucleator compounds is generally accompanied by a deprotonation reaction or a hydrolysis reaction, as opposed to a bond cleavage reaction.

The emulsion layer of the photographic element of the invention can comprise any one or more of the light sensitive layers of the photographic element. The photographic elements made in accordance with the present invention can be black and white elements, single color elements or multi-color elements. Multicolor elements contain dye image-forming units sensitive to each of the three primary regions of the spectrum. Each unit can be comprised of a single emulsion layer or of multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

A typical multicolor photographic element comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. The element can contain additional layers, such as filter layers, interlayers, overcoat layers, subbing layers, and the like. All of these can be coated on a support which can be transparent or reflective (for example, a paper support).

Photographic elements of the present invention may also usefully include a magnetic recording material as described in *Research Disclosure*, Item 34390, November 1992, or a transparent magnetic recording layer such as a layer containing magnetic particles on the underside of a transparent support as in U.S. Pat. No. 4,279,945 and U.S. Pat. No. 4,302,523. The element typically will have a total thickness (excluding the support) of from 5 to 30 microns. While the order of the color sensitive layers can be varied, they will normally be red-sensitive, green-sensitive and blue-

sensitive, in that order on a transparent support, (that is, blue sensitive furthest from the support) and the reverse order on a reflective support being typical.

The present invention also contemplates the use of photographic elements of the present invention in what are often referred to as single use cameras (or "film with lens" units). These cameras are sold with film preloaded in them and the entire camera is returned to a processor with the exposed film remaining inside the camera. Such cameras may have glass or plastic lenses through which the photographic element is exposed.

In the following discussion of suitable materials for use in elements of this invention, reference will be made to *Research Disclosure*, September 1994, Number 365, Item 36544, which will be identified hereafter by the term

15 "Research Disclosure I." The Sections hereafter referred to are Sections of the Research Disclosure I unless otherwise indicated. All Research Disclosures referenced are published by Kenneth Mason Publications, Ltd., Dudley Annex, 12a North Street, Emsworth, Hampshire PO10 7DQ, ENGLAND. The foregoing references and all other references cited in this application, are incorporated herein by reference.

The silver halide emulsions employed in the photographic elements of the present invention may be negative-working, 25 such as surface-sensitive emulsions or unfogged internal latent image forming emulsions, or positive working emulsions of internal latent image forming emulsions (that are either fogged in the element or fogged during processing). Suitable emulsions and their preparation as well as methods 30 of chemical and spectral sensitization are described in Sections I through V. Color materials and development modifiers are described in Sections V through XX. Vehicles which can be used in the photographic elements are described in Section II, and various additives such as 35 brighteners, antifoggants, stabilizers, light absorbing and scattering materials, hardeners, coating aids, plasticizers, lubricants and matting agents are described, for example, in Sections VI through XIII. Manufacturing methods are described in all of the sections, layer arrangements particularly in Section XI, exposure alternatives in Section XVI, and processing methods and agents in Sections XIX and XX.

With negative working silver halide a negative image can be formed. Optionally a positive (or reversal) image can be formed although a negative image is typically first formed.

45 The photographic elements of the present invention may also use colored couplers (e.g. to adjust levels of interlayer correction) and masking couplers such as those described in EP 213 490; Japanese Published Application 58-172,647; U.S. Pat. No. 2,983,608; German Application DE 2,706, 50 117C; U.K. Patent 1,530,272; Japanese Application A-1 13935; U.S. Pat. No. 4,070,191 and German Application DE 2,643,965. The masking couplers may be shifted or blocked.

The photographic elements may also contain materials 55 that accelerate or otherwise modify the processing steps of bleaching or fixing to improve the quality of the image. Bleach accelerators described in EP 193 389; EP 301 477; U.S. Pat. No. 4,163,669; U.S. Pat. No. 4,865,956; and U.S. Pat. No. 4,923,784 are particularly useful. Also contemplated is the use of nucleating agents, development accelerators or their precursors (UK Patent 2,097,140; U.K. Patent 2,131,188); development inhibitors and their precursors (U.S. Pat. No. 5,460,932; U.S. Pat. No. 5,478,711); electron transfer agents (U.S. Pat. No. 4,859,578; U.S. Pat. No. 4,912,025); antifogging and anti color-mixing agents such as derivatives of hydroquinones, aminophenols, amines, gallic acid; catechol; ascorbic acid; hydrazides; sulfonamidophenols; and non color-forming couplers.

The elements may also contain filter dye layers comprising colloidal silver sol or yellow and/or magenta filter dyes and/or antihalation dyes (particularly in an undercoat beneath all light sensitive layers or in the side of the support opposite that on which all light sensitive layers are located) either as oil-in-water dispersions, latex dispersions or as solid particle dispersions. Additionally, they may be used with "smearing" couplers (e.g. as described in U.S. Pat. No. 4,366,237; EP 096 570; U.S. Pat. No. 4,420,556; and U.S. Pat. No. 4,543,323.) Also, the couplers may be blocked or coated in protected form as described, for example, in Japanese Application 61/258,249 or U.S. Pat. No. 5,019,492.

The photographic elements may further contain other image-modifying compounds such as "Development Inhibitor-Releasing" compounds (DIR's). Useful additional DIR's for elements of the present invention, are known in the art and examples are described in U.S. Pat. Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publication: 272,573; 335,319; 336,411; 346,899; 362,870; 365,252; 365,346; 373,382; 376,212; 377,463; 378,236; 384,670; 396,486; 401,612; 401,613.

DIR compounds are also disclosed in "Developer-Inhibitor-Releasing (DIR) Couplers for Color Photography," C. R. Barr, J. R. Thirtle and P. W. Vittum in *Photographic Science and Engineering*, Vol. 13, p. 174 (1969), incorporated herein by reference.

It is also contemplated that the concepts of the present invention may be employed to obtain reflection color prints as described in *Research Disclosure*, November 1979, Item 18716, available from Kenneth Mason Publications, Ltd, Dudley Annex, 12a North Street, Emsworth, Hampshire P0101 7DQ, England, incorporated herein by reference. The emulsions and materials to form elements of the present invention, may be coated on pH adjusted support as described in U.S. Pat. No. 4,917,994; with epoxy solvents (EP 0 164 961); with additional stabilizers (as described, for example, in U.S. Pat. No. 4,346,165; U.S. Pat. No. 4,540,653 and U.S. Pat. No. 4,906,559); with ballasted chelating agents such as those in U.S. Pat. No. 4,994,359 to reduce sensitivity to polyvalent cations such as calcium; and with stain reducing compounds such as described in U.S. Pat. No. 5,068,171 and U.S. Pat. No. 5,096,805. other compounds which may be useful in the elements of the invention are disclosed in Japanese Published Applications 83-09,959; 83-62,586; 90-072,629; 90-072,630; 90-072,632; 90-072,633; 90-072,634; 90-077,822; 90-078,229; 90-078,230; 90-079,336; 90-079,338; 90-079,690; 90-079,691; 90-080,487; 90-080,489; 90-080,490; 90-080,491; 90-080,492; 90-080,494; 90-085,928; 90-086,669; 90-086,670; 90-087,361; 90-087,362; 90-087,363; 90-087,364; 90-088,096; 90-088,097; 90-093,662; 90-093,663; 90-093,664; 90-093,665; 90-093,666; 90-093,668; 90-094,055; 90-094,056; 90-101,937; 90-103,409; 90-151,577.

The silver halide used in the photographic elements may be silver iodobromide, silver bromide, silver chloride, silver chlorobromide, silver chloroiodobromide, and the like.

The type of silver halide grains preferably include polymorphic, cubic, and octahedral. The grain size of the silver halide may have any distribution known to be useful in photographic compositions, and may be either polydispersed or monodispersed.

Tabular grain silver halide emulsions may also be used. Tabular grains are those with two parallel major faces each clearly larger than any remaining grain face and tabular grain emulsions are those in which the tabular grain, account for at least 30 percent, more typically at least 50 percent, preferably >70 percent and optimally >90 percent of total grain projected area. The tabular grains can account for substantially all (>97 percent) of total grain projected area. The tabular grain emulsions can be high aspect ratio tabular grain emulsions—i.e.,  $ECD/t > 8$ , where ECD is the diameter of a circle having an area equal to grain projected area and t is tabular grain thickness; intermediate aspect ratio tabular grain emulsions—i.e.,  $ECD/t = 5$  to 8; or low aspect ratio tabular grain emulsions—i.e.,  $ECD/t = 2$  to 5. The emulsions typically exhibit high tabularity (T), where T (i.e.,  $ECD/t^2$ ) > 25 and ECD and t are both measured in micrometers (mm). The tabular grains can be of any thickness compatible with achieving an aim average aspect ratio and/or average tabularity of the tabular grain emulsion. Preferably the tabular grains satisfying projected area requirements are those having thicknesses of <0.3 mm, thin (<0.2 mm) tabular grains being specifically preferred and ultrathin (<0.07 mm) tabular grains being contemplated for maximum tabular grain performance enhancements. When the native blue absorption of iodohalide tabular grains is relied upon for blue speed, thicker tabular grains, typically up to 0.5 mm in thickness, are contemplated.

High iodide tabular grain emulsions are illustrated by House U.S. Pat. No. 4,490,458, Maskasky U.S. Pat. No. 4,459,353 and Yagi et al EPO 0 410 410.

Tabular grains formed of silver halide(s) that form a face centered cubic (rock salt type) crystal lattice structure can have either {100} or {111} major faces. Emulsions containing {111} major face tabular grains, including those with controlled grain dispersities, halide distributions, twin plane spacing, edge structures and grain dislocations as well as adsorbed {111} grain face stabilizers, are illustrated in those references cited in *Research Disclosure I*, Section I.B.(3) (page 503).

The silver halide grains to be used in the invention may be prepared according to methods known in the art, such as those described in *Research Disclosure I* and James, *The Theory of the Photographic Process*. These include methods such as ammoniacal emulsion making, neutral or acidic emulsion making, and others known in the art. These methods generally involve mixing a water soluble silver salt with a water soluble halide salt in the presence of a protective colloid, and controlling the temperature, pAg, pH values, etc., at suitable values during formation of the silver halide by precipitation.

In the course of grain precipitation one or more dopants (grain occlusions other than silver and halide) can be introduced to modify grain properties. For example, any of the various conventional dopants disclosed in *Research Disclosure*, Item 36544, Section I. Emulsion grains and their preparation, sub-section G. Grain modifying conditions and adjustments, paragraphs (3), (4) and (5), can be present in the emulsions of the invention. In addition it is specifically contemplated to dope the grains with transition metal hexa-coordination complexes containing one or more organic ligands, as taught by Olm et al U.S. Pat. No. 5,360,712, the disclosure of which is here incorporated by reference.

It is specifically contemplated to incorporate in the face centered cubic crystal lattice of the grains a dopant capable of increasing imaging speed by forming a shallow electron trap (hereinafter also referred to as a SET) as discussed in Research Disclosure Item 36736 published November 1994, here incorporated by reference.

The SET dopants are effective at any location within the grains. Generally better results are obtained when the SET dopant is incorporated in the exterior 50 percent of the grain, based on silver. An optimum grain region for SET incorporation is that formed by silver ranging from 50 to 85 percent of total silver forming the grains. The SET can be introduced all at once or run into the reaction vessel over a period of time while grain precipitation is continuing. Generally SET forming dopants are contemplated to be incorporated in concentrations of at least  $1 \times 10^{-7}$  mole per silver mole up to their solubility limit, typically up to about  $5 \times 10^{-4}$  mole per silver mole.

SET dopants are known to be effective to reduce reciprocity failure. In particular the use of iridium hexacoordination complexes or  $\text{Ir}^{+4}$  complexes as SET dopants is advantageous.

Iridium dopants that are ineffective to provide shallow electron traps (non-SET dopants) can also be incorporated into the grains of the silver halide grain emulsions to reduce reciprocity failure.

To be effective for reciprocity improvement the Ir can be present at any location within the grain structure. A preferred location within the grain structure for Ir dopants to produce reciprocity improvement is in the region of the grains formed after the first 60 percent and before the final 1 percent (most preferably before the final 3 percent) of total silver forming the grains has been precipitated. The dopant can be introduced all at once or run into the reaction vessel over a period of time while grain precipitation is continuing. Generally reciprocity improving non-SET Ir dopants are contemplated to be incorporated at their lowest effective concentrations.

The contrast of the photographic element can be further increased by doping the grains with a hexacoordination complex containing a nitrosyl or thionitrosyl ligand (NZ dopants) as disclosed in McDugle et al U.S. Pat. No. 4,933,272, the disclosure of which is here incorporated by reference.

The contrast increasing dopants can be incorporated in the grain structure at any convenient location. However, if the NZ dopant is present at the surface of the grain, it can reduce the sensitivity of the grains. It is therefore preferred that the NZ dopants be located in the grain so that they are separated from the grain surface by at least 1 percent (most preferably at least 3 percent) of the total silver precipitated in forming the silver iodochloride grains. Preferred contrast enhancing concentrations of the NZ dopants range from  $1 \times 10^{-11}$  to  $4 \times 10^{-8}$  mole per silver mole, with specifically preferred concentrations being in the range from  $10^{-10}$  to  $10^{-8}$  mole per silver mole.

Although generally preferred concentration ranges for the various SET, non-SET Ir and NZ dopants have been set out above, it is recognized that specific optimum concentration ranges within these general ranges can be identified for specific applications by routine testing. It is specifically contemplated to employ the SET, non-SET Ir and NZ dopants singly or in combination. For example, grains containing a combination of an SET dopant and a non-SET Ir dopant are specifically contemplated. Similarly SET and NZ dopants can be employed in combination. Also NZ and Ir dopants that are not SET dopants can be employed in

combination. Finally, the combination of a non-SET Ir dopant with a SET dopant and an NZ dopant. For this latter three-way combination of dopants it is generally most convenient in terms of precipitation to incorporate the NZ dopant first, followed by the SET dopant, with the non-SET Ir dopant incorporated last.

The photographic elements of the present invention, as is typical, provide the silver halide in the form of an emulsion. Photographic emulsions generally include a vehicle for coating the emulsion as a layer of a photographic element. Useful vehicles include both naturally occurring substances such as proteins, protein derivatives, cellulose derivatives (e.g., cellulose esters), gelatin (e.g., alkali-treated gelatin such as cattle bone or hide gelatin, or acid treated gelatin such as pigskin gelatin), gelatin derivatives (e.g., acetylated gelatin, phthalated gelatin, and the like), and others as described in *Research Disclosure I*. Also useful as vehicles or vehicle extenders are hydrophilic water-permeable colloids. These include synthetic polymeric peptizers, carriers, and/or binders such as poly(vinyl alcohol), poly(vinyl lactams), acrylamide polymers, polyvinyl acetals, polymers of alkyl and sulfoalkyl acrylates and methacrylates, hydrolyzed polyvinyl acetates, polyamides, polyvinyl pyridine, methacrylamide copolymers, and the like, as described in *Research Disclosure I*. The vehicle can be present in the emulsion in any amount useful in photographic emulsions. The emulsion can also include any of the addenda known to be useful in photographic emulsions.

The silver halide to be used in the invention may be advantageously subjected to chemical sensitization. Compounds and techniques useful for chemical sensitization of silver halide are known in the art and described in *Research Disclosure I* and the references cited therein. Compounds useful as chemical sensitizers, include, for example, active gelatin, sulfur, selenium, tellurium, gold, platinum, palladium, iridium, osmium, rhenium, phosphorous, or combinations thereof. Chemical sensitization is generally carried out at pAg levels of from 5 to 10, pH levels of from 4 to 8, and temperatures of from 30 to 80° C., as described in *Research Disclosure I*, Section IV (pages 510-511) and the references cited therein.

The silver halide may be sensitized by sensitizing dyes by any method known in the art, such as described in *Research Disclosure I*. The dye may be added to an emulsion of the silver halide grains and a hydrophilic colloid at any time prior to (e.g., during or after chemical sensitization) or simultaneous with the coating of the emulsion on a photographic element. The dyes may, for example, be added as a solution in water or an alcohol. The dye/silver halide emulsion may be mixed with a dispersion of color image-forming coupler immediately before coating or in advance of coating (for example, 2 hours).

Photographic elements of the present invention are preferably imagewise exposed using any of the known techniques, including those described in *Research Disclosure I*, section XVI. This typically involves exposure to light in the visible region of the spectrum, and typically such exposure is of a live image through a lens, although exposure can also be exposure to a stored image (such as a computer stored image) by means of light emitting devices (such as light emitting diodes, CRT and the like).

Photographic elements comprising the composition of the invention can be processed in any of a number of well-known photographic processes utilizing any of a number of well-known processing compositions, described, for example, in *Research Disclosure I*, or in T. H. James, editor, *The Theory of the Photographic Process*, 4th Edition,

Macmillan, New York, 1977. In the case of processing a negative working element, the element is treated with a color developer (that is one which will form the colored image dyes with the color couplers), and then with an oxidizer and a solvent to remove silver and silver halide. In the case of processing a reversal color element, the element is first treated with a black and white developer (that is, a developer which does not form colored dyes with the coupler compounds) followed by a treatment to fog silver halide (usually chemical fogging or light fogging), followed by treatment with a color developer. Preferred color developing agents are p-phenylenediamines. Especially preferred are: 4-amino N,N-diethylaniline hydrochloride, 4-amino-3-methyl-N,N-diethylaniline hydrochloride, 4-amino-3-methyl-N-ethyl-N-(b-(methanesulfonamido)ethylaniline sesquisulfate hydrate, 4-amino-3-methyl-N-ethyl-N-(b-hydroxyethyl)aniline sulfate, 4-amino-3-b-(methanesulfonamido)ethyl-N,N-diethylaniline hydrochloride and 4-amino-N-ethyl-N-(2-methoxyethyl)-m-toluidine di-p-toluene sulfonic acid.

Dye images can be formed or amplified by processes which employ in combination with a dye-image-generating reducing agent an inert transition metal-ion complex oxidizing agent, as illustrated by Bissonette U.S. Pat. Nos. 3,748,138, 3,826,652, 3,862,842 and 3,989,526 and Travis U.S. Pat. No. 3,765,891, and/or a peroxide oxidizing agent as illustrated by Matejec U.S. Pat. No. 3,674,490, *Research Disclosure*, Vol. 116, December, 1973, Item 11660, and Bissonette *Research Disclosure*, Vol. 148, August, 1976, Items 14836, 14846 and 14847. The photographic elements can be particularly adapted to form dye images by such processes as illustrated by Dunn et al et al U.S. Pat. No. 3,822,129, Bissonette U.S. Pat. Nos. 3,834,907 and 3,902, 905, Bissonette et al U.S. Pat. No. 3,847,619, Mowrey U.S. Pat. No. 2,904,413, Hirai et al U.S. Pat. No. 4,880,725, Iwano U.S. Pat. No. 4,954,425, Marsden et al U.S. Pat. No. 4,983,504, Evans et al U.S. Pat. No. 5,246,822, Twist U.S. Pat. No. 5,324,624, Fyson EPO 0 487 616, Tannahill et al WO 90/13059, Marsden et al WO 90/13061, Grimsey et al WO 91/16666, Fyson WO 91/17479, Marsden et al WO 92/01972. Tannahill WO 92/05471, Henson WO 92/07299, Twist WO 93/01524 and WO 93/11460 and Wingender et al German OLS 4,211,460.

Development is followed by bleach-fixing, to remove silver or silver halide, washing and drying.

The fragmentable electron donating sensitizer compounds of the present invention can be included in a silver halide emulsion by direct dispersion in the emulsion, or they may be dissolved in a solvent such as water, methanol or ethanol for example, or in a mixture of such solvents, and the resulting solution can be added to the emulsion. The compounds of the present invention may also be added from solutions containing a base and/or surfactants, or may be incorporated into aqueous slurries or gelatin dispersions and then added to the emulsion. The compounds are generally used together with conventional sensitizing dye, and can be added before, during or after the addition of the conventional sensitizing dye.

The amount of fragmentable electron donating compound which is employed in this invention may range from as little as  $1 \times 10^{-8}$  to as much as about  $2 \times 10^{-3}$  mole per mole of silver in an emulsion layer. More preferably the concentra-

tion of the compounds is from about  $5 \times 10^{-7}$  to about  $2 \times 10^{-4}$  mole per mole of silver in an emulsion layer. Where the oxidation potential  $E_1$  for the XY group of the fragmentable two-electron donating sensitizer is a relatively low potential, it is more active, and relatively less agent need be employed. Conversely, where the oxidation potential for the XY group of the fragmentable two-electron donating sensitizer is relatively high, a larger amount thereof, per mole of silver, is employed. For fragmentable one-electron donating sensitizers relatively larger amounts per mole of silver are also employed.

Conventional spectral sensitizing dyes can be used in combination with the fragmentable electron donor of this invention. Preferred sensitizing dyes that can be used are cyanine dyes, complex cyanine dyes, merocyanine dyes, complex merocyanine dyes, styryl dyes, and hemicyanine dyes. Illustrative sensitizing dyes that can be used are dyes of the following general structures (XII)–(XVI):

(XII)



wherein:

$E_1$ ,  $J$ ,  $q$ ,  $p$ , and  $D_1$  are defined as set forth above, and  $E_4$  is defined the same as  $E_1$ ,  $r$  represents 0 or 1, and  $D_2$  is defined the same as  $D_1$ ;

(XIII)



wherein  $E_1$ ,  $D_1$ ,  $J$ ,  $p$ ,  $q$  and  $W_2$  are as defined above for formula (XII) and  $G$  represents



wherein  $E_2$ ,  $F$ , and  $F'$  are as defined above in formula (IX);

(XIV)



wherein  $D_1$ ,  $E_1$ ,  $J$ ,  $p$ ,  $q$  and  $W_2$  are as defined above for formula (XII), and  $G_2$  represents a substituted or unsubstituted amino group or a substituted or unsubstituted aryl group;



wherein D<sub>1</sub>, E<sub>1</sub>, D<sub>2</sub>, E<sub>4</sub>, J, p, q, r and W<sub>2</sub> are as defined for formula (XII) and (XIII) above, and E<sub>3</sub> is as defined for formula (X) above;



wherein D<sub>1</sub>, E<sub>1</sub>, J, G, p, q, r and W<sub>2</sub> are as defined above for formula (XV) above and E<sub>3</sub> is as defined for formula (X) above.

In the above formulas, E<sub>1</sub> and E<sub>4</sub> each independently represents the atoms necessary to complete a substituted or unsubstituted 5- or 6-membered heterocyclic nucleus. These include a substituted or unsubstituted: thiazole nucleus, oxazole nucleus, selenazole nucleus, quinoline nucleus, tellurazole nucleus, pyridine nucleus, thiazoline nucleus, indoline nucleus, oxadiazole nucleus, thiadiazole nucleus, or imidazole nucleus. This nucleus may be substituted with known substituents, such as halogen (e.g., chloro, fluoro, bromo), alkoxy (e.g., methoxy, ethoxy), substituted or unsubstituted alkyl (e.g., methyl, trifluoromethyl), substituted or unsubstituted aryl, substituted or unsubstituted aralkyl, sulfonate, and others known in the art.

In one embodiment of the invention, when dyes according to formula (XII) are used E<sub>1</sub> and E<sub>4</sub> each independently represent the atoms necessary to complete a substituted or unsubstituted thiazole nucleus, a substituted or unsubstituted selenazole nucleus, a substituted or unsubstituted imidazole nucleus, or a substituted or unsubstituted oxazole nucleus.

Examples of useful nuclei for E<sub>1</sub> and E<sub>4</sub> include: a thiazole nucleus, e.g., thiazole, 4-methylthiazole, 4-phenylthiazole, 5-methylthiazole, 5-phenylthiazole, 4,5-dimethyl-thiazole, 4,5-diphenylthiazole, 4-(2-thienyl)thiazole, benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 5-phenylbenzothiazole, 6-phenylbenzothiazole, 4-methoxybenzothiazole, 5-methoxybenzothiazole, 6-methoxybenzothiazole, 4-ethoxybenzothiazole, 5-ethoxybenzothiazole, tetrahydrobenzothiazole, 5,6-dimethoxybenzothiazole, 5,6-dioxymethylbenzothiazole, 5-hydroxybenzothiazole, 6,5-dihydroxybenzothiazole, naphtho[2,1-d]thiazole, 5-ethoxynaphtho[2,3-d]thiazole, 8-methoxynaphtho[2,3-d]thiazole, 7-methoxynaphtho[2,3-d]thiazole, 4'-methoxythianaphtho-7',6'-4,5-thiazole, etc.; an oxazole nucleus, e.g., 4-methyloxazole, 5-methyloxazole, 4-phenyloxazole, 4,5-diphenyloxazole, 4-ethyloxazole, 4,5-dimethyloxazole, 5-phenyloxazole, benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-ethoxybenzoxazole, 5-chlorobenzoxazole,

- 10 6-methoxybenzoxazole, 5-hydroxybenzoxazole, naphtho[2,1-d]oxazole, naphtho[1,2-d]oxazole, etc.; a selenazole nucleus, e.g., 4-methylselenazole, 4-phenylselenazole, benzoselenazole, 5-chlorobenzoselenazole, 5-methoxybenzoselenazole, 15 5-hydroxybenzoselenazole, tetrahydrobenzoselenazole, naphtho[2,1-d]selenazole, naphtho[1,2-d]selenazole, etc.; a pyridine nucleus, e.g., 2-pyridine, 5-methyl-2-pyridine, 4-pyridine, 3-methyl-4-pyridine, 3-methyl-4-pyridine, etc.; a quinoline nucleus, e.g., 2-quinoline, 3-methyl-2-quinoline, 5-ethyl-2-quinoline, 6-chloro-2-quinoline, 8-chloro-2-quinoline, 6-methoxy-2-quinoline, 8-hydroxy-2-quinoline, 4-quinoline, 6-methoxy-4-quinoline, 7-methyl-4-quinoline, 8-chloro-4-quinoline, etc.; a tellurazole nucleus, e.g., benzotellurazole, naphtho[1,2-d]benzotellurazole, 5,6-dimethoxybenzotellurazole, 5-methoxybenzotellurazole, 5-methylbenzotellurazole; a thiazoline nucleus, e.g., thiazoline, 4-methylthiazoline, etc.; a benzimidazole nucleus, e.g., benzimidazole, 5-trifluoromethylbenzimidazole, 5,6-dichlorobenzimidazole; and indole nucleus, 3,3-dimethylindole, 3,3-diethylindole, 3,3,5-trimethylindole; or a diazole nucleus, e.g., 5-phenyl-1,3,4-oxadiazole, 5-methyl-1,3,4-thiadiazole.
- F and F' are each a cyano radical, an ester radical such as 35 ethoxy carbonyl, methoxycarbonyl, etc., an acyl radical, a carbamoyl radical, or an alkylsulfonyl radical such as ethylsulfonyl, methylsulfonyl, etc. Examples of useful nuclei for E<sub>2</sub> include a 2-thio-2,4-oxazolidinedione nucleus (i.e., those of the 2-thio-2,4-(3H,5H)-oxaazolidinone series) 40 (e.g., 3-ethyl-2-thio-2,4 oxazolidinedione, 3-(2-sulfoethyl)-2-thio-2,4 oxazolidinedione, 3-(4-sulfonyl)-2-thio-2,4 oxazolidinedione, 3-(3-carboxypropyl)-2-thio-2,4 oxazolidinedione, etc.; a thianaphthenone nucleus (e.g., 2-(2H)-thianaphthenone, etc.), a 2-thio-2,5-thiazolidinedione nucleus (i.e., the 2-thio-2,5-(3H,4H)-thiazoledeione series) (e.g., 3-ethyl-2-thio-2,5-thiazolidinedione, etc.); a 2,4-thiazolidinedione nucleus (e.g., 2,4-thiazolidinedione, 3-ethyl-2,4-thiazolidinedione, 3-phenyl-2,4-thiazolidinedione, 3-a-naphthyl-2,4-thiazolidinedione, etc.); a thiazolidinone nucleus (e.g., 4-thiazolidinone, 3-ethyl-4-thiazolidinone, 3-phenyl-4-thiazolidinone, 3-a-naphthyl-4-thiazolidinone, etc.); a 2-thiazolin-4-one series (e.g., 2-ethylmercapto-2-thiazolin-4-one, 2-alkylphenylamino-2-thiazolin-4-one, 2-diphenylamino-2-thiazolin-4-one, etc.) a 2-imino-4-oxazolidinedione (i.e., pseudohydantoin) series (e.g., 2,4-imidazolidinedione, 3-ethyl-2,4-imidazolidinedione, 3-phenyl-2,4-imidazolidinedione, 3-a-naphthyl-2,4-imidazolidinedione, 1,3-diethyl-2,4-imidazolidinedione, 1-ethyl-3-phenyl-2,4-imidazolidinedione, 1-ethyl-2-anaphthyl-2,4-imidazolidinedione, 1,3-diphenyl-2,4-imidazolidinedione, etc.); a 2-thio-2,4-imidazolidinedione (i.e., 2-thiohydantoin) nucleus (e.g., 2-thio-2,4-imidazolidinedione, 3-ethyl-2-thio-2,4-imidazolidinedione, 3-(2-carboxyethyl)-2-thio-2,4-imidazolidinedione, 3-phenyl-2-thio-2,4-imidazolidinedione, 1,3-diethyl-2-thio-

**49**

2,4-imidazolidinedione, 1-ethyl-3-phenyl -2-thio-2,4-imidazolidinedione, 1-ethyl-3-naphthyl-2-thio-2,4-imidazolidinedione, 1,3-diphenyl-2-thio-2,4-imidazolidinedione, etc.); a 2-imidazolin-5-one nucleus.

G2 represents a substituted or unsubstituted amino radical (e.g., primary amino, anilino), or a substituted or unsubstituted aryl radical (e.g., phenyl, naphthyl, dialkylaminophenyl, tolyl, chlorophenyl, nitrophenyl).

According to the formulas (VIII)–(XII), each J represents a substituted or unsubstituted methine group. Examples of substituents for the methine groups include alkyl (preferably of from 1 to 6 carbon atoms, e.g., methyl, ethyl, etc.) and aryl (e.g., phenyl). Additionally, substituents on the methine groups may form bridged linkages.

W2 represents a counterion as necessary to balance the charge of the dye molecule. Such counterions include cations and anions for example sodium, potassium, triethylammonium, tetramethylguanidinium, diisopropylammonium and tetrabutylammonium, chloride, bromide, iodide, para-toluene sulfonate and the like.

**50**

D1 and D2 are each independently substituted or unsubstituted aryl (preferably of 6 to 15 carbon atoms), or more preferably, substituted or unsubstituted alkyl (preferably of from 1 to 6 carbon atoms). Examples of aryl include phenyl, tolyl, p-chlorophenyl, and p-methoxyphenyl. Examples of alkyl include methyl, ethyl, propyl, isopropyl, butyl, hexyl, cyclohexyl, decyl, dodecyl, etc., and substituted alkyl groups (preferably a substituted lower alkyl containing from 1 to 6 carbon atoms), such as a hydroxyalkyl group, e.g., 2-hydroxyethyl, 4-hydroxybutyl, etc., a carboxyalkyl group, e.g., 2-carboxyethyl, 4-carboxybutyl, etc., a sulfoalkyl group, e.g., 2-sulfoethyl, 3-sulfobutyl, 4-sulfobutyl, etc., a sulfatoalkyl group, etc., an acyloxyalkyl group, e.g., 2-acetoxyethyl, 3-acetoxypropyl, 4-butyroxybutyl, etc., an alkoxy carbonylalkyl group, e.g., 2-methoxycarbonyl ethyl, 4-ethoxycarbonylbutyl, etc., or an aralkyl group, e.g., benzyl, phenethyl, etc. The alkyl or aryl group may be substituted by one or more of the substituents on the above-described substituted alkyl groups.

Particularly preferred dyes are:

Dye 1



Dye 2



Dye 3



-continued

Dye 4



Dye 5



Dye 6



Dye 7



Dye 8





Dye 10



Dye 11



Dye 12



Dye 13





and



Dye 19



Dye 20

The ratio of conventional spectral sensitizing dye to the fragmentable electron donating sensitizing agent of the present invention, which may be determined through an ordinary emulsion test, is typically from about 99.99:0.01 to about 50:50 by mol.

Various compounds may be added to the photographic material of the present invention for the purpose of lowering the fogging of the material during manufacture, storage, or processing. Typical antifoggants are discussed in Section VI of Research Disclosure I, for example tetraazaindenes, mercaptotetrazoles, polyhydroxybenzenes, hydroxyaminobenzenes, combinations of a thiosulfonate and a sulfonate, and the like.

For this invention, polyhydroxybenzene and hydroxyaminobenzene compounds (hereinafter "hydroxybenzene compounds") are preferred as they are effective for lowering fog without decreasing the emulsion sensitivity. Examples of hydroxybenzene compounds are:



In these formulae, V and V' each independently represent —H, —OH, a halogen atom, —OM (M is alkali metal ion), an alkyl group, a phenyl group, an amino group, a carbonyl

group, a sulfone group, a sulfonated phenyl group, a sulfonated alkyl group, a sulfonated amino group, a carboxyphenyl group, a carboxyalkyl group, a carboxyamino group, a hydroxyphenyl group, a hydroxyalkyl group, an alkylether group, an alkylphenyl group, an alkylthioether group, or a phenylthioether group.

More preferably, they each independently represent —H, —OH, —Cl, —Br, —COOH, —CH<sub>2</sub>CH<sub>2</sub>COOH, —CH<sub>3</sub>, —CH<sub>2</sub>CH<sub>3</sub>, —C(CH<sub>3</sub>)<sub>3</sub>, —OCH<sub>3</sub>, —CHO, —SO<sub>3</sub>K, —SO<sub>3</sub>Na, —SO<sub>3</sub>H, —SCH<sub>3</sub>, or —phenyl.

Especially preferred hydroxybenzene compounds follow:





35 Hydroxybenzene compounds may be added to the emulsion layers or any other layer constituting the photographic material of the present invention. The preferred amount added is from  $1 \times 10^{-3}$  to  $1 \times 10^{-1}$  mol, and more preferred is  $1 \times 10^{-3}$  to  $2 \times 10^{-2}$  mol, per mol of silver halide.

40 Laser Flash Photolysis Method

(a) Oxidation Potential of Radical X•

The laser flash photolysis measurements were performed using a nanosecond pulsed excimer (Questek model 2620, 308 nm, ca. 20 ns, ca. 100 mJ) pumped dye laser (Lambda

45 Physik model FL 3002). The laser dye was DPS (commercially available from Exciton Co.) in p-dioxane (410 nm, ca. 20 ns, ca. 10 mJ). The analyzing light source was a pulsed 150 W xenon arc lamp (Osram XBO 150/W). The arc lamp power supply was a PRA model 302 and the

50 pulser was a PRA model M-306. The pulser increased the light output by ca. 100 fold, for a time period of ca. 2–3 ms. The analyzing light was focused through a small aperture (ca. 1.5 mm) in a cell holder designed to hold 1 cm<sup>2</sup> cuvettes. The laser and analyzing beams irradiated the cell from

55 opposite directions and crossed at a narrow angle (ca. 15°). After leaving the cell, the analyzing light was collimated and focused onto the slit (1 mm, 4 nm bandpass) of an ISA H-20 monochromator. The light was detected using 5 dynodes of a Hamamatsu model R446 photomultiplier. The output of

60 the photomultiplier tube was terminated into 50 ohm, and captured using a Tektronix DSA-602 digital oscilloscope. The entire experiment is controlled from a personal computer.

The experiments were performed either in acetonitrile, or

65 a mixture of 80% acetonitrile and 20% water. The first singlet excited state of a cyanoanthracene (A), which acted as the electron acceptor, was produced using the nanosecond

laser pulse at 410 nm. Quenching of this excited state by electron transfer from the relatively high oxidation potential donor biphenyl (B), resulted in efficient formation of separated, "free", radical ions in solution,  $A^- + B^+$ . Secondary electron transfer then occurred between  $B^+$  and the lower oxidation potential electron donor X-Y, to generate  $X-Y^+$  in high yield. For the investigations of the oxidation potentials of the radicals  $X^*$ , typically the cyanoanthracene concentration was ca.  $2 \times 10^{-5}$  M to  $10^{-4}$  M, the biphenyl concentration was ca. 0.1 M. The concentration of the X-Y donor was ca.  $10^{-3}$  M. The rates of the electron transfer reactions are determined by the concentrations of the substrates. The concentrations used ensured that the  $A^-$  and the  $X-Y^+$  were generated within 100 ns of the laser pulse. The radical ions could be observed directly by means of their visible absorption spectra. The kinetics of the photogenerated radical ions were monitored by observation of the changes in optical density at the appropriate wavelengths.

The reduction potential ( $E_{red}$ ) of 9,10-dicyanoanthracene (DCA) is  $-0.91$  V. In a typical experiment, DCA is excited and the initial photoinduced electron transfer from the biphenyl (B) to the DCA forms a  $DCA^-$ , which is observed at its characteristic absorption maximum ( $\lambda_{obs} = 705$  nm), within ca. 20 ns of the laser pulse. Rapid secondary electron transfer occurs from X-Y to  $B^+$  to generate  $X-Y^+$ , which fragments to give  $X^*$ . A growth in absorption is then observed at 705 nm with a time constant of ca. 1 microsecond, due to reduction of a second DCA by the  $X^*$ . The absorption signal with the microsecond growth time is equal to the size of the absorption signal formed within 20 ns. If reduction of two DCA was observed in such an experiment, this indicates that the oxidation potential of the  $X^*$  is more negative than  $-0.9$  V.

If the oxidation potential of  $X^*$  is not sufficiently negative to reduce DCA, an estimate of its oxidation potential was obtained by using other cyanoanthracenes as acceptors. Experiments were performed in an identical manner to that described above except that 2,9,10-tricyanoanthracene (TriCA,  $E_{red} = -0.67$  V,  $\lambda_{obs} = 710$  nm) or tetracyanoanthracene (TCA,  $E_{red} = -0.44$  V,  $\lambda_{obs} = 715$  nm) were used as the electron acceptors. The oxidation potential of the  $X^*$  was taken to be more negative than  $-0.7$  if reduction of two TriCA was observed, and more negative than  $-0.5$  V if reduction of two TCA was observed. Occasionally the size of the signal from the second reduced acceptor was smaller than that of the first. This was taken to indicate that electron transfer from the  $X^*$  to the acceptor was barely exothermic, i.e. the oxidation potential of the radical was essentially the same as the reduction potential of the acceptor.

To estimate the oxidation potentials of  $X^*$  with values less negative than  $-0.5$  V, i.e. not low enough to reduce even tetracyanoanthracene, a slightly different approach was used. In the presence of low concentrations of an additional acceptor, Q, that has a less negative reduction potential than the primary acceptor, A (DCA, for example), secondary electron transfer from  $A^-$  to Q will take place. If the reduction potential of Q is also less negative than the oxidation potential of the  $X^*$ , then Q will also be reduced by the radical, and the magnitude of the  $Q^-$  absorption signal will be doubled. In this case, both the first and the second electron transfer reactions are diffusion controlled and occur at the same rate. Consequently, the second reduction cannot be time resolved from the first. Therefore, to determine

whether two electron reduction actually takes place, the  $Q^-$  signal size must be compared with an analogous system for which it is known that reduction of only a single Q occurs. For example, a reactive  $X-Y^+$  which might give a reducing  $X^*$  can be compared with a nonreactive  $X-Y^+$ . Useful secondary electron acceptors (Q) that have been used are chlorobenzoquinone ( $E_{red} = -0.34$  V,  $\lambda_{obs} = 450$  nm), 2,5-dichlorobenzoquinone ( $E_{red} = -0.18$  V,  $\lambda_{obs} = 455$  nm) and 2,3,5,6-tetrachlorobenzoquinone ( $E_{red} = 0.00$  V,  $\lambda_{obs} = 460$  nm).

#### (b) Fragmentation Rate Constant Determination

The laser flash photolysis technique was also used to determine fragmentation rate constants for examples of the oxidized donors X-Y. The radical cations of the X-Y donors absorb in the visible region of the spectrum. Spectra of related compounds can be found in "Electron Absorption Spectra of Radical Ions" by T. Shida, Elsevier, New York, 1988. These absorptions were used to determine the kinetics of the fragmentation reactions of the radical cations of the X-Y. Excitation of 9,10-dicyanoanthracene (DCA) in the presence of biphenyl and the X-Y donor, as described above, results in the formation of the  $DCA^-$  and the  $X-Y^+$ . By using a concentration of X-Y of ca.  $10^{-2}$  M, the  $X-Y^+$  can be formed within ca. 20 ns of the laser pulse. With the monitoring wavelength set within an absorption band of the  $X-Y^+$ , a decay in absorbance as a function of time is observed due to the fragmentation reaction. The monitoring wavelengths used were somewhat different for the different donors, but were mostly around 470–530 nm. In general the  $DCA^-$  also absorbed at the monitoring wavelengths, however, the signal due to the radical anion was generally much weaker than that due to the radical cation, and on the timescale of the experiment the  $A^-$  did not decay, and so did not contribute to the observed kinetics. As the  $X-Y^+$  decayed, the radical  $X^*$  was formed, which in most cases reacted with the cyanoanthracene to form a second  $A^-$ . To make sure that this "grow-in" of absorbance due to  $A^-$  did not interfere with the time-resolved decay measurements, the concentration of the cyanoanthracene was maintained below ca.  $2 \times 10^{-5}$  M. At this concentration the second reduction reaction occurred on a much slower timescale than the  $X-Y^+$  decay. Alternatively, when the decay rate of the  $X-Y^+$  was less than  $10^6$  s $^{-1}$ , the solutions were purged with oxygen. Under these conditions the  $DCA^-$  reacted with the oxygen to form  $O_2^-$  within 100 ns, so that its absorbance did not interfere with that of the  $X-Y^+$  on the timescale of its decay.

The experiments measuring the fragmentation rate constants were performed in acetonitrile with the addition of 20% water, so that all of the salts could be easily solubilized. Most experiments were performed at room temperature. In some cases the fragmentation rate was either too fast or too slow to be easily determined at room temperature. When this happened, the fragmentation rate constants were measured as a function of temperature, and the rate constant at room temperature determined by extrapolation.

Typical examples of the synthesis of compounds Q-XY follow. Other compounds can also be synthesized by analogy using appropriate selected known starting materials. The following compounds are synthesized by reaction Scheme I.



**Preparation of Intermediate A, R<sub>1</sub>—CH<sub>3</sub>**

Aniline (21.4 g, 230 mmol), potassium iodide (4.6 g), ethyl 2-bromopropionate (50.0 g, 276 mmol) and potassium carbonate (82.8 g, 599 mmol) were added to 300 mL of acetonitrile and the mixture was heated at reflux under nitrogen for 2 days. The solution was cooled, and the precipitated salt was removed by filtration. The filtrate was partitioned between dichloromethane and aqueous sodium bicarbonate. The organic layer was separated, washed with water, dried over anhydrous sodium sulfate and concentrated at reduced pressure. Fractional vacuum distillation of the resulting oil provided the desired intermediate A (31.9 g, 72%) with bp 108–115° C. at 0.05 mm.

**Preparation of Intermediate B, R<sub>1</sub>—CH<sub>3</sub>; R<sub>2</sub>'—CH<sub>2</sub>CO<sub>2</sub>t-Bu**

Aniline (126.7 g, 1.36 mol), t-butyl acrylate (174.5 g, 1.36 mol) and methane sulfonic acid (4 mL) were combined and stirred at reflux for 4 h. The mixture was then cooled and ligroin (1 L) was then added. The resulting precipitate was removed by filtration. The filtrate was concentrated at reduced pressure and the residue subjected to fractional vacuum distillation, bp 115–125° C. at 0.3–0.5 mm, 138 g, 46%.

A mixture of t-butyl 3-phenylaminopropionate (170 g, 0.77 mol), potassium carbonate (106 g, 0.77 mol), ethyl 2-bromopropionate (139 g, 0.77 mol) and 1200 mL of butyronitrile were heated at reflux for 18 hours. An additional 0.23 mole of potassium carbonate and ethyl

<sup>40</sup> 2-bromopropionate were added to help drive the reaction to completion and the mixture was heated at reflux for 24 hours. The reaction mixture was cooled, filtered, and the filtrate was concentrated at reduced pressure. The resulting oil was subjected to fractional vacuum distillation. The desired product had a bp of 170–185° C. at 0.05 mm, and 138 g (56%) was isolated.

**Preparation of Intermediate C, R<sub>1</sub>—CH<sub>3</sub>; R<sub>2</sub>'—CH<sub>2</sub>CO<sub>2</sub>tBu**

Dimethylformamide (DMF) (20 mL) was cooled to 0° C. and POCl<sub>3</sub> (2 mL) was added slowly. The mixture was stirred for 1 hour at 0° C., warmed briefly to rt, and then recooled to 0° C. The ester (B, R<sub>1</sub>—CH<sub>3</sub>; R<sub>2</sub>'—CH<sub>2</sub>CO<sub>2</sub>tBu) (2.0 g) was dissolved in 2 mL DMF and added slowly. The solution was allowed to warm to rt, and was stirred at this temperature 18 hours. The reaction mixture was then cooled to 0° C and 50 mL of saturated aq. sodium acetate was added. The solution was then added to 100 mL of ether and the aqueous phase was separated. The organic phase was washed three times with 100 mL of brine, dried over anhydrous sodium sulfate and concentrated at reduced pressure. The resulting oil was charged onto a silica gel column and eluted with heptane:THF (3:1). The desired aldehyde was isolated as a light yellow oil (1.6 g, 74%).

**Preparation of Intermediate C, R<sub>1</sub>—CH<sub>3</sub>; R<sub>2</sub>'—CH<sub>2</sub>CO<sub>2</sub>H**

The ester (C, R<sub>1</sub>—CH<sub>3</sub>; R<sub>2</sub>'—CH<sub>2</sub>CO<sub>2</sub>tBu, 1.6 g) was dissolved in 10 mL trifluoroacetic acid (TFA) and was stirred 18 hours at room temperature. The TFA was removed at reduced pressure and the resulting oil was subjected to a

**65**

pressure of 0.01 mm for 10 hours to remove all residual TFA. The remaining oil was used without further purification.

Preparation of Intermediate D,  $R_1=CH_3$ ;  $R_2=CH_2CO_2Na$

The ester ( $R_1=CH_3$ ;  $R_2=CH_2CO_2H$ , 2.0g, 6.8 mmol) was dissolved in 10 mL ethanol and 1N sodium hydroxide (13.6 mmol) was added. The reaction mixture was stirred 18 hours at room temperature and then concentrated at reduced pressure. The resulting white solid (2.0 g) was used without purification.

Preparation of INV 1,  $R_1=CH_3$ ;  $R_2=CH_2CO_2Na$ ,  $X=H$

The aldehyde (D,  $R_1=CH_3$ ;  $R_2=CH_2CO_2Na$ , 0.8 g, 2.6 mmol), and 3-ethyl-2-methyl benzothiazolium p-toluenesulfonate (0.9 g, 2.6 mmol) were dissolved in 20 mL ethanol and the mixture was stirred 18 hours at room temperature. The solvent was removed at reduced pressure and the resulting purple solid was chromatographed on silica gel using methanol as the eluant, yielding the INV 1 (0.3 g, 27%).

Preparation of INV 3,  $R_1=CH_3$ ;  $R_2=CH_2CO_2Na$ ,  $X=Cl$

The aldehyde (D,  $R_1=CH_3$ ;  $R_2=CH_2CO_2Na$ , 0.3 g, 1.0 mmol) and 5-chloro-3-ethyl-2-methyl benzothiazolium p-toluenesulfonate (0.39 g, 1.0 mmol) were dissolved in 5 mL ethanol and the mixture was stirred 18 h at room temperature. The solvent was removed at reduced pressure and the resulting purple solid was chromatographed on silica gel using methanol as the eluant, yielding the INV 3 (0.18g, 40%).

Preparation of Intermediate B,  $R_1=CH_3$ ;  $R_2'=CO_2Et$

The ester A ( $R_1=CH_3$ ) (24.6 g, 127 mmol), ethyl bromoacetate (31.9 g, 191 mmol), potassium carbonate (26.0 g, 190 mmol) and potassium iodide (cat. amt.) were added to 200 mL of acetonitrile and heated at reflux under nitrogen for 6 days. The reaction mixture was cooled and the precipitated salt filtered. The filtrate was dissolved in dichloromethane, washed with aqueous sodium bicarbonate and water. The organic phase was then dried over anhydrous sodium sulfate and concentrated at reduced pressure. The resulting oil was fractionally distilled under vacuum to give B,  $R_1=CH_3$ ;  $R_2'=CO_2Et$  (20.8 g, 58%, bp 138–142° C., 0.028 mm).

Preparation of Intermediate C,  $R_1=CH_3$ ;  $R_2'=CO_2Et$

Dimethylformamide (DMF) (20 mL) was cooled to 0° C. and  $POCl_3$  (2 mL) was added slowly. The mixture was stirred for 1 hour at 0° C., warmed briefly to rt, and then re-cooled to 0° C. The ester (B,  $R_1=CH_3$ ;  $R_2'=CO_2Et$ ) (2.0 g) was dissolved in 2 mL DMF and added slowly. The solution was allowed to warm to rt, and was stirred at this temperature 18 hours. The reaction mixture was then cooled to 0° C. and 50 mL of saturated aq. sodium acetate was added. The solution was then added to 100 mL of ether and the aqueous phase was separated. The organic phase was washed three times with 100 mL of brine, dried over anhydrous sodium sulfate and concentrated at reduced pressure. The resulting oil was charged onto a silica gel column and eluted with heptane:THF (1:1). The desired aldehyde was isolated as a light yellow oil (1.8 g, 82%).

Preparation of Intermediate D,  $R_1=CH_3$ ;  $R_2=CO_2Na$

The ester ( $R_1=CH_3$ ;  $R_2'=CO_2Et$ , 1.0 g, 3.2 mmol) was dissolved in 5 mL ethanol and 1N sodium hydroxide (6.5 mmol) was added. The reaction mixture was stirred 18 hours at room temperature and then concentrated at reduced pressure. The resulting white solid (1.0 g) was used without purification.

Preparation of INV 2,  $R_1=CH_3$ ;  $R_2=CO_2Na$ ,  $X=Cl$

The aldehyde (D,  $R_1=CH_3$ ;  $R_2=CO_2Na$ , 0.3 g, 1.0 mmol) and 5-chloro-3-ethyl-2-methyl benzothiazolium

**66**

p-toluenesulfonate (0.39 g, 1.0 mmol) were dissolved in 10 mL ethanol and the mixture was stirred 6 h at room temperature. The solvent was removed at reduced pressure and the resulting purple solid was chromatographed on silica gel using methanol as the eluant, yielding the INV 2 (0.15 g, 36%).

Preparation of Intermediate B,  $R_1=CH_3$ ;  $R_2'=Ph$

The ester A ( $R_1=CH_3$ ) (3.8 g, 20 mmol), benzyl chloride (2.6 g, 21 mmol), and lutidine (2.5 g, 23 mmol) were dissolved in 25 mL of acetonitrile and heated at reflux for 36 hours. The solution was then partitioned between 200 mL of ethyl acetate and 100 mL of brine. The organic layer was separated, dried over anhydrous sodium sulfate and concentrated at reduced pressure. The resulting oil was charged onto a silica gel column and eluted with heptane:THF (4:1). The desired product was isolated as a colorless oil (2.0 g, 36%).

Preparation of Intermediate C,  $R_1=CH_3$ ;  $R_2'=Ph$

Dimethylformamide (DMF) (20 mL) was cooled to 0° C. and  $POCl_3$  (2 mL) was added slowly. The mixture was stirred for 1 hour at 0° C., warmed briefly to rt, and then re-cooled to 0° C. The ester (B,  $R_1=CH_3$ ;  $R_2'=Ph$ ) (2.0 g) was dissolved in 2 mL DMF and added slowly. The solution was allowed to warm to rt, and was stirred at this temperature 18 hours. The reaction mixture was then cooled to 0° C. and 50 mL of saturated aq. sodium acetate was added. The solution was then added to 100 mL of ether and the aqueous phase was separated. The organic phase was washed three times with 100 mL of brine, dried over anhydrous sodium sulfate and concentrated at reduced pressure. The resulting oil was charged onto a silica gel column and eluted with heptane:THF (4:1). The desired aldehyde was isolated as a light yellow oil (1.6 g, 73%).

Preparation of Intermediate D,  $R_1=CH_3$ ;  $R_2=Ph$

The ester C ( $R_1=CH_3$ ;  $R_2=Ph$ , 1.4 g, 4.5 mmol) was dissolved in 25 mL methanol and 1N sodium hydroxide (4.5 mmol) was added. The reaction mixture was stirred 18 hours at room temperature and then concentrated at reduced pressure. The resulting white solid (1.4 g) was used without purification.

Preparation of INV 4,  $R_1=CH_3$ ;  $R_2=Ph$ ,  $X=Cl$

The aldehyde (D,  $R_1=CH_3$ ;  $R_2=Ph$ , 0.6 g, 2.0 mmol) and 5-chloro-3-ethyl-2-methyl benzothiazolium p-toluenesulfonate (0.76 g, 2.0 mmol) were dissolved in 5 mL ethanol and the mixture was stirred 6 h at room temperature. The solvent was removed at reduced pressure and the resulting purple solid was chromatographed on silica gel using methanol as the eluant, yielding the INV 4 (0.07 g, 7%).

Preparation of Intermediate B,  $R_1=CH_3$ ;  $R_2'=CN$

The ester A ( $R_1=CH_3$ ) (3.8 g, 20 mmol), bromoacetonitrile (2.5 g, 20 mmol), and lutidine (2.5 g, 23 mmol) were dissolved in 25 mL of acetonitrile and the mixture was heated at reflux for 36 hours. The solution was then partitioned between 200 mL ethyl acetate and 100 mL brine. The organic layer was separated, dried over anhydrous sodium sulfate and concentrated at reduced pressure. The resulting oil was charged onto a silica gel column and eluted with heptane:THF (4:1). The desired product was isolated as a colorless oil (3.0 g, 65%).

Preparation of Intermediate C,  $R=CH_3$ ;  $R_2'=CN$

Dimethylformamide (DMF) (30 mL) was cooled to 0° C. and  $POCl_3$  (3 mL) was added slowly. The mixture was stirred for 1 hour at 0° C., warmed briefly to rt, and then re-cooled to 0° C. The ester (B,  $R_1=CH_3$ ;  $R_2'=CN$ ) (3.0 g) was dissolved in 2 mL DMF and added slowly. The solution was allowed to warm to rt, and was stirred at this temperature 18 hours. The reaction mixture was then cooled to 0° C.

and 50 mL of saturated aq. sodium acetate was added. The solution was then added to 100 mL of ether and the aqueous phase was separated. The organic phase was washed three times with 100 mL of brine, dried over anhydrous sodium sulfate and concentrated at reduced pressure. The resulting oil was charged onto a silica gel column and eluted with heptane:THF (4:1). The desired aldehyde was isolated as a light yellow oil (1.1 g, 32%).

Preparation of Intermediate D,  $R_1=CH_3$ ;  $R_2=CONH_2$

The ester C ( $R_1=CH_3$ ;  $R_2=CN$ , 1.1 g, 4.2 mmol) was dissolved in 20 mL methanol and 1N sodium hydroxide (4.2 mmol) was added. The reaction mixture was stirred 18 hours at room temperature and then concentrated at reduced pressure. The resulting white solid (0.9 g) was used without purification.

Preparation of INV 5,  $R_1=CH_3$ ;  $R_2=CONH_2$ ,  $X=Cl$

The aldehyde (D,  $R_1=CH_3$ ;  $R_2=CONH_2$ , 0.9 g, 3.5 mmol) and 5-chloro-3-ethyl-2-methyl benzothiazolium p-toluene sulfonate (1.3 g, 3.5 mmol) were dissolved in 5 mL ethanol and the mixture was stirred 18 h at room temperature. The solvent was removed at reduced pressure and the resulting purple solid was chromatographed on silica gel using methanol as the eluent, yielding the INV 5 (0.5 g, 32%).

Preparation of Intermediate B,  $R_1=CH_3$ ;  $R_2=CF_3$

The ester A ( $R_1=CH_3$ ) (1.0 g, 5.2 mmol), trifluoroethyltriflate (1.2 g, 5.2 mmol) and lutidine (1.0 g, 9.3 mmol) were heated in a sealed tube at 135° C. for 48 hours. The tube contents were then partitioned between ethyl acetate and brine. The organic layer was separated, dried over anhydrous sodium sulfate and concentrated at reduced pressure. The resulting oil was chromatographed on silica gel using heptane:THF as eluent (4:1). 0.5 g (35%) of the desired product was isolated.

Preparation of Intermediate C,  $R_1=CH_3$ ;  $R_2=CF_3$

Dimethylformamide (DMF) (30 mL) was cooled to 0° C. and  $POCl_3$  (3 mL) was added slowly. The mixture was stirred for 1 hour at 0° C., warmed briefly to rt, and then recooled to 0° C. The ester (B,  $R_1=CH_3$ ;  $R_2=CF_3$ ) (1.0 g) was dissolved in 2 mL DMF and added slowly. The solution was allowed to warm to rt, and was stirred at this temperature 18 hours. The reaction mixture was then cooled to 0° C. and 50 mL of saturated aq. sodium acetate was added. The solution was then added to 100 mL of ether and the aqueous phase was separated. The organic phase was washed three times with 100 mL of brine, dried over anhydrous sodium sulfate and concentrated at reduced pressure. The resulting oil was charged onto a silica gel column and eluted with

heptane:THF (1:1). The desired aldehyde was isolated as a light yellow oil (0.5 g, 45%).

Preparation of Intermediate D,  $R_1=CH_3$ ;  $R_2=CF_3$

The ester C ( $R_1=CH_3$ ;  $R_2=CF_3$ , 0.87 g, 2.9 mmol) was dissolved in 10 mL methanol and 1N sodium hydroxide (2.9 mmol) was added. The reaction mixture was stirred 18 hours at room temperature and then concentrated at reduced pressure. The resulting white solid (0.9 g) was used without purification.

Preparation of INV 7,  $R_1=CH_3$ ;  $R_2=CF_3$ ,  $X=Cl$

The aldehyde (D,  $R_1=CH_3$ ;  $R_2=CF_3$ , 0.9 g, 3 mmol) and 5-chloro-3-ethyl-2-methyl benzothiazolium p-toluene sulfonate (1.2 g, 3.0 mmol) were dissolved in 5 mL ethanol and the mixture was stirred 18 h at room temperature. The solvent was removed at reduced pressure and the resulting solid was chromatographed on silica gel using methanol as the eluent, yielding the INV 7 (0.1 g, 7%).

Preparation of Intermediate C,  $R_1=H$ ;  $R_2=CH_3$

Dimethylformamide (DMF) (400 mL) was cooled to 0° C. and  $POCl_3$  (40 mL) was added slowly. The mixture was stirred for 1 hour at 0° C., warmed briefly to rt, and then recooled to 0° C. The ester (B,  $R_1=H$ ;  $R_2=CH_3$ ) (42 g) was dissolved in 20 mL DMF and added slowly. The solution was allowed to warm to rt, and was stirred at this temperature 18 hours. The reaction mixture was then cooled to 0° C. and 500 mL of saturated aq. sodium acetate was added. The solution was then added to 500 mL of ether and the aqueous phase was separated. The organic phase was washed three times with 100 mL of brine, dried over anhydrous sodium sulfate and concentrated at reduced pressure. The resulting oil was charged onto a silica gel column and eluted with heptane:THF (1:1). The desired aldehyde was isolated as a light yellow oil (25 g, 52%).

Preparation of Intermediate D,  $R_1=H$ ;  $R_2=CH_3$

The ester C ( $R_1=H$ ;  $R_2=CH_3$ , 5 g, 23 mmol) was dissolved in 50 mL methanol and 1N sodium hydroxide (23 mmol) was added. The reaction mixture was stirred 18 hours at room temperature and then concentrated at reduced pressure. The resulting white solid (5 g) was used without purification.

Preparation of INV 6,  $R_1=H$ ;  $R_2=CH_3$ ,  $X=Cl$

The aldehyde (D,  $R_1=H$ ;  $R_2=CH_3$ , 2.3 g, 10 mmol) and 5-chloro-3-ethyl-2-methyl benzothiazolium p-toluene sulfonate (3.8 g, 10 mmol) were dissolved in 25 mL ethanol and the mixture was stirred 18 h at room temperature. The solvent was removed at reduced pressure and the resulting solid was chromatographed on silica gel using methanol as the eluent, yielding the INV 6 (0.4 g, 10%).

INV 42 was synthesized according to reaction Scheme II

Scheme II





#### Preparation of Intermediate E

5-Methylamino-2-methylbenzothiazole (10.7 g, 60 mmol), ethyl-2-bromopropionate (21.7 g, 120 mmol), and potassium carbonate (16.6 g, 120 mmol) were added to 500 mL of butyronitrile and the mixture was heated at reflux for 52 hours. The mixture was cooled and the precipitated salt was removed by filtration. The solvent was removed from the filtrate by evaporation at reduced pressure. The light brown viscous material was purified by flash chromatography on a silica gel column eluting with heptane/ethyl acetate (3/2). The desired product was obtained as a colorless viscous liquid (yield 16.0 g).

#### Preparation of Intermediate F

Intermediate E (12.4 g, 45 mmol), 1,2-propane sulfone (6.6 g, 54 mmol), and 1-methyl-2-pyrrolidinone (100 mL) were combined and stirred and heated at 160° C. for 16 hours. The mixture was cooled and the solvent was removed with a rotary evaporator. The dark colored residue was dissolved in a methylene chloride/methanol (95/5) mixture and chromatographed on silica gel yielding 4.2 g of the desired product.

#### Preparation of Intermediate H

Intermediate F (4.0 g, 10 mmol), intermediate G (3.34 g, 10 mmol), 80 mL glacial acetic acid, and 10 mL of acetic anhydride were combined, stirred, and heated on an oil bath for 5 minutes at 50° C. The heat was removed and 20 mL of

pyridine was added, and the mixture was stirred to 10 minutes, then the mixture was heated with stirring at 50° C. for 1 hour. The solvent was then completely removed using a rotary evaporator, and the resultant brown residue was triturated with acetone, ether, and pentane. The dark yellow solid was filtered and washed with pentane (100 mL). The solid was dried in a vacuum oven, and then purified by flash chromatography using methylene chloride/methanol (85/15) mixture as the eluent to give 0.95 g of the desired product. Preparation of INV 42

Intermediate H (0.66 g, 0.86 mmol), sodium hydroxide (0.08 g, 2 mmol), methanol (200 mL), and water (100 mL) were combined and stirred at room temperature for 2 days. The solvent was removed at reduced pressure and the brown residue was triturated with methanol (20 mL). The insoluble material was filtered and washed successively with acetone, ether, and pentane. The solid was dried in a vacuum oven at room temperature to give 0.56 g of INV 42.

Examples illustrating the beneficial use of these fragmentable electron donating sensitizer compounds in silver halide emulsions are given in the following:

#### EXAMPLE 1

An AgBrI tabular silver halide emulsion (Emulsion T-1) was prepared containing 4.05% total I distributed such that the central portion of the emulsion grains contained 1.5% I

and the perimeter area contained substantially higher I as described by Chang et. al., U.S. Pat. No. No. 5,314,793. The emulsion grains had an average thickness of 0.103  $\mu\text{m}$  and average circular diameter of 1.25  $\mu\text{m}$ . Emulsion T-1 was precipitated using deionized gelatin. The emulsion was sulfur sensitized by adding 1,3-dicarboxymethyl-1,3-dimethyl-2-thiourea at 40° C.; the temperature was then raised to 60° C. at a rate of 5° C./3 min and the emulsions held for 20 min before cooling to 40° C. The amounts of the sulfur sensitizing compound used was  $8.5 \times 10^{-6}$  mole/mole Ag. The chemically sensitized emulsion was then used to prepare the experimental coating variations indicated in Table I.

All of these experimental coating variations contained the hydroxybenzene, 2,4-disulfocatechol (HB3) at a concentration of 13 mmole/mole Ag, added to the melt before any further addenda. The fragmentable electron donating sensitizer (FED) compound was dissolved in methanol solution and added to the emulsion at the relative concentrations indicated in Table I. At the time of FED sensitizer addition, the emulsion melts had a VAg of 85–90 mV and a pH of 6.0. After 5 min at 40° C., additional water, gelatin, and surfactant were then added to the emulsion melts to give a final emulsion melt that contained 216 grams of gel per mole of silver. These emulsion melts were coated onto an acetate film base at 1.61 g/m<sup>2</sup> of Ag with gelatin at 3.22 g/m<sup>2</sup>. The coatings were prepared with a protective overcoat which contained gelatin at 1.08 g/m<sup>2</sup>, coating surfactants, and a bisvinylsulfonylmethyl ether as a gelatin hardening agent.

For photographic evaluation, each of the coating strips was exposed for 0.1 sec to a 365 nm emission line of a Hg lamp filtered through a Kodak Wratten filter number 18A and a step wedge ranging in density from 0 to 4 density units in 0.2 density steps. The exposed film strips were developed for 6 min in Kodak Rapid X-ray Developer (KRX).  $S_{365}$ , relative sensitivity at 365 nm, was evaluated at a density of 0.15 units above fog.

The data in Table I compare the photographic sensitivities for an undyed emulsion containing the fragmentable electron donating sensitizer compound INV 1. For this exposure, relative sensitivity was set equal to 100 for the control emulsion coating with no fragmentable electron donating sensitizer agent added (test no. 1). Improved sensitivity for the 365 nm exposure was shown for the examples which contained the fragmentable electron donating sensitizing agent (test nos. 2–5). The data in Table I show that INV 1 gave up to a factor of 1.6 sensitivity increase relative to the control. Only minor increases in fog accompanied these sensitivity increases.

TABLE I

| Speed and fog results for INV 1 on Emulsion T-1 |                                     |                          |      |           |
|-------------------------------------------------|-------------------------------------|--------------------------|------|-----------|
| Test No.                                        | Amount of INV 1 added (mmol/mol Ag) | Photographic Sensitivity |      |           |
|                                                 |                                     | $S_{365}$                | Fog  | Remarks   |
| 1                                               | none                                | 100                      | 0.05 | control   |
| 2                                               | 0.046                               | 146                      | 0.19 | invention |
| 3                                               | 0.091                               | 164                      | 0.11 | invention |
| 4                                               | 0.182                               | 160                      | 0.13 | invention |
| 5                                               | 0.364                               | 150                      | 0.1  | invention |

## EXAMPLE 2

The sulfur sensitized emulsion T-1 as described in Example 1 was used to prepare coatings containing combi-

nations of the fragmentable electron-donating sensitizing agents listed in Table II and blue spectral sensitizing dye D-I or green spectral sensitizing dye D-II. These experimental coating variations contained the hydroxybenzene 2,4-disulfocatechol (HB3) at a concentration of 13 mmole/mole Ag, added to the melt before the addition of any sensitizing dye compounds. The total concentration of dye used, that is the sum of the amounts of conventional spectral sensitizer plus fragmentable electron donating sensitizer, was 0.91 mmole/mole Ag for coatings containing the dye D-I and 0.86 mmole/mole Ag for coatings containing the dye D-II. The sensitizing dye and fragmentable electron donating compounds were added to the emulsion at 40° C. and the coatings were prepared as described in Example 1.

For photographic evaluation, each of the coating strips was exposed for 0.1 sec to a 365 nm emission line of a Hg lamp filtered through a Kodak Wratten filter number 18A and a step wedge ranging in density from 0 to 4 density units in 0.2 density steps. The exposed film strips were developed for 6 min in Kodak Rapid X-ray Developer (KRX).  $S_{365}$ , relative sensitivity at 365 nm, was evaluated at a density of 0.15 units above fog. For the 365 nm exposure, relative sensitivity was set equal to 100 for the control emulsion coating (test no. 1) with no dye or fragmentable electron donating sensitizer agent added.

The data in Table II compare the photographic sensitivities for emulsions containing various combinations of fragmentable electron donating sensitizer compounds with a conventional blue or green spectral sensitizing dye. The addition of conventional sensitizing dyes D-I or D-II cause some sensitivity decrease for the 365 nm exposure relative to the undyed control (tests nos. 2 and 10) due to desensitization. Improved sensitivity for the 365 nm exposure was shown for the examples which contained mixtures of D-I and a fragmentable electron donating sensitizer agent (test nos. 3–9). The data in Table II show that Inv 1–7 gave a factor of 1.6 to 1.8 sensitivity increase relative to the comparison emulsion coating containing only D-I. No increase in fog accompanied these sensitivity increases. Sensitivity increases  $S_{365}$  relative to the comparison (test no 10) of up to factor of 1.6 were also found when the fragmentable electron donating sensitizer is used in combination with a conventional green sensitizing dye (test nos. 11–17), showing that the fragmentable electron donating sensitizer is effective in ameliorating dye desensitization. However, somewhat larger increases in fog were obtained with the inventive compounds when the green sensitizing dye D-II was present. These fog increases are minimal when the XY portion of the fragmentable electron donating sensitizer contains an electron withdrawing group such as the  $\text{CF}_3\text{CH}_2-$  or  $\text{CONH}_2-$  groups as indicated in the structure of INV 5 and INV 7.

Additional testing was carried out to determine the response of the coatings that contained the green spectral sensitizing dye D-II to a spectral exposure. The coating strips (from test nos. 10, 12, 15, and 17) were exposed for 0.1 sec to a 3000K color temperature tungsten lamp filtered to give an effective color temperature of 5500K and further filtered through a Kodak Wratten filter number 9 and a step wedge ranging in density from 0 to 4 density units in 0.2 density steps. This filter passes only light of wavelengths longer than 460 nm, thus giving light absorbed mainly by the green sensitizing dye II. The exposed film strips were developed for 6 min in Kodak Rapid X-ray Developer (KRX).  $S_{WR9}$ , relative sensitivity for this Kodak Wratten filter 9 exposure, was evaluated at a density of 0.15 units above fog. For this spectral exposure, the relative sensitivity

was set equal to 100 for the control coating with no fragmentable electron donating compound added.

-continued

D-II



The data of Table II show that sensitivity advantages were obtained for both intrinsic exposures of the silver halide at 365 nm and spectral exposures of the green sensitizing dye, using the Kodak Wratten 9 filter. Sensitivity  $S_{WR9}$  increases relative to the comparison of a factor of 1.3 to 1.4 were obtained for the experimental coatings containing the fragmentable electron donating sensitizer compounds INV 2, INV 5, and INV 7. Overall, these results show that these fragmentable electron donating sensitizers can remove dye desensitization caused by conventional sensitizing dyes, and can also give additional increases in photographic sensitivity.

TABLE II

| Test | Type of         | Total Amount of<br>Sensitizing Dye<br>and FED added | Amount of FED<br>in mixture<br>% of total |          | Photographic<br>Sensitivity |           |      | Remarks    |
|------|-----------------|-----------------------------------------------------|-------------------------------------------|----------|-----------------------------|-----------|------|------------|
|      |                 |                                                     | Type of                                   | Dye conc | $S_{365}$                   | $S_{WR9}$ | Fog  |            |
| No.  | Sensitizing Dye | (mmol/mol Ag)                                       | FED                                       |          |                             |           |      |            |
| 1    | none            |                                                     | control                                   | 0        | 100                         | —         | 0.03 | control    |
| 2    | D-I             | 0.91                                                | none                                      | 0        | 95                          | —         | 0.04 | comparison |
| 3    | D-I             | 0.91                                                | INV 1                                     | 1%       | 170                         | —         | 0.04 | invention  |
| 4    | D-I             | 0.91                                                | INV 2                                     | 1%       | 158                         | —         | 0.04 | invention  |
| 5    | D-I             | 0.91                                                | INV 3                                     | 1%       | 170                         | —         | 0.04 | invention  |
| 6    | D-I             | 0.91                                                | INV 4                                     | 1%       | 170                         | —         | 0.04 | invention  |
| 7    | D-I             | 0.91                                                | INV 5                                     | 1%       | 155                         | —         | 0.03 | invention  |
| 8    | D-I             | 0.91                                                | INV 6                                     | 1%       | 151                         | —         | 0.04 | invention  |
| 9    | D-I             | 0.91                                                | INV 7                                     | 1%       | 151                         | —         | 0.03 | invention  |
| 10   | D-II            | 0.86                                                | none                                      | 0        | 81                          | 100       | 0.06 | comparison |
| 11   | D-II            | 0.86                                                | INV 1                                     | 0.5%     | —                           | —         | 0.76 | invention  |
| 12   | D-II            | 0.86                                                | INV 2                                     | 0.5%     | 129                         | 138       | 0.12 | invention  |
| 13   | D-II            | 0.86                                                | INV 3                                     | 0.5%     | —                           | —         | 1.00 | invention  |
| 14   | D-II            | 0.86                                                | INV 4                                     | 0.5%     | —                           | —         | 0.93 | invention  |
| 15   | D-II            | 0.86                                                | INV 5                                     | 0.5%     | 120                         | 132       | 0.08 | invention  |
| 16   | D-II            | 0.86                                                | INV 6                                     | 0.5%     | —                           | —         | 0.59 | invention  |
| 17   | D-II            | 0.86                                                | INV 7                                     | 0.5%     | 126                         | 141       | 0.09 | invention  |

### EXAMPLE 3

The chemically sensitized AgBrI tabular emulsion T-1 described in Example I was used to prepare the experimental 50 coating variations listed in Table III, comparing various fragmentable two-electron donors to structurally related compounds that do not fragment. The inventive and comparison compounds were added to the emulsion, and coatings prepared and tested as described in example 1.



55 The compounds INV 1, INV 5, and INV 7 in the Table III contain the fragmentable electron donating moiety XY. As indicated in commonly assigned, copending patent application Ser. No. 08/740,536 filed Oct. 30, 1996, the entire disclosure of which is incorporated herein by reference, the 60 XY groups in these sensitizing agents have one electron oxidation potentials  $E_1$  which are less positive than 1.4 V and upon oxidation, fragment to give  $CO_2$  and a corresponding neutral radical, and the neutral radical has an oxidation potential equal to or more negative than -0.7 V. For the 65 365 nm exposure, the data of Table III illustrates that for the coatings containing the blue spectral sensitizing dye D-I, the fragmentable two-electron donor compounds INV 1 and

INV 7 gave large sensitivity increases, of a factor of greater than 1.6. These sensitivity gains could be obtained with only minor increases in fog levels. In contrast, the comparison compounds COMP 1 and COMP 2, which are derivatives of INV 1 and INV 7 wherein the carboxylate functional group is replaced by an ethyl ester group, do not undergo a fragmentation reaction when oxidized and give very little or no sensitivity increase. Likewise, related compounds such as comparison compounds COMP 4-COMP 10 which contain a hemicyanine chromophore but do not contain an XY group, give very little or no increase in emulsion sensitivity.

Similarly, the comparison compounds COMP 4-COMP 10 give very little or no sensitivity increase in coatings containing the emulsion with the green sensitizing dye II. On the other hand, INV 5 and INV 7 gave sensitivity increases of a factor of greater than 1.4 on the coatings with the green sensitizing dye II.

fragmentable electron donating sensitizing agent INV 1 was added to the emulsion in two ways: as an additional component in the chemical sensitization procedure, added after the dyes D-I and D-III and the PMT antifoggant, or during the melt preparation after the addition of the antifoggant tetraazaindene. The variations examined are given in Table IV.

The melts were prepared for coating by adding the antifoggant and stabilizer tetraazaindene at 1.25 gm per mole Ag, additional water, and gelatin. Coatings were prepared by combining the emulsion melts with a melt containing gelatin, coating surfactants, and an aqueous dispersion of the yellow-forming color couplers YY-1 and YY-2 and coating the resulting mixture on acetate support. The final coatings contained Ag at 0.86 g/m<sup>2</sup>, YY-1 coupler at 1.08 g/m<sup>2</sup>, YY-2 coupler at 0.03 g/m<sup>2</sup>, and gelatin at 3.22 g/m<sup>2</sup>. The coatings were overcoated with a protective layer

TABLE III

Speed and fog results for combinations of FED and blue or green sensitizing dye on Emulsion T-1

| Test | Type of Sensitizing | Total Amount of Sensitizing Dye and compound added | Type of compound | Amount of FED or COMP in mixture % of total | Photographic Sensitivity |                  |            |
|------|---------------------|----------------------------------------------------|------------------|---------------------------------------------|--------------------------|------------------|------------|
|      |                     |                                                    |                  |                                             | Dye conc                 | S <sub>365</sub> | Fog        |
| No.  | Dye                 | (mmol/mol Ag)                                      | added            |                                             |                          |                  | Remarks    |
| 1    | none                |                                                    | control          | 0                                           | 100                      | 0.04             | control    |
| 2    | D-I                 | 0.91                                               | none             | 0                                           | 98                       | 0.04             | comparison |
| 3    | D-I                 | 0.91                                               | COMP 4           | 1%                                          | 100                      | 0.04             | comparison |
| 4    | D-I                 | 0.91                                               | COMP 5           | 1%                                          | 98                       | 0.04             | comparison |
| 5    | D-I                 | 0.91                                               | COMP 6           | 1%                                          | 100                      | 0.04             | comparison |
| 6    | D-I                 | 0.91                                               | COMP 8           | 3%                                          | 100                      | 0.04             | comparison |
| 7    | D-I                 | 0.91                                               | COMP 7           | 3%                                          | 98                       | 0.03             | comparison |
| 8    | D-I                 | 0.91                                               | COMP 9           | 1%                                          | 93                       | 0.04             | comparison |
| 9    | D-I                 | 0.91                                               | COMP 10          | 1%                                          | 100                      | 0.05             | comparison |
| 10   | D-I                 | 0.91                                               | INV 1            | 1%                                          | 182                      | 0.06             | invention  |
| 11   | D-I                 | 0.91                                               | COMP 1           | 1%                                          | 95                       | 0.04             | comparison |
| 12   | D-I                 | 0.91                                               | COMP 2           | 1%                                          | 98                       | 0.04             | comparison |
| 13   | D-I                 | 0.91                                               | INV 7            | 1%                                          | 158                      | 0.05             | invention  |
| 14   | D-II                | 0.86                                               | none             | 0                                           | 91                       | 0.06             | comparison |
| 15   | D-II                | 0.86                                               | COMP 4           | 1%                                          | 93                       | 0.06             | comparison |
| 16   | D-II                | 0.86                                               | COMP 5           | 1%                                          | 89                       | 0.06             | comparison |
| 17   | D-II                | 0.86                                               | COMP 6           | 1%                                          | 89                       | 0.06             | comparison |
| 18   | D-II                | 0.86                                               | COMP 8           | 1%                                          | 89                       | 0.06             | comparison |
| 19   | D-II                | 0.86                                               | COMP 7           | 1%                                          | 91                       | 0.06             | comparison |
| 20   | D-II                | 0.86                                               | COMP 10          | 1%                                          | 91                       | 0.06             | comparison |
| 21   | D-II                | 0.86                                               | INV 1            | 0.1%                                        | —                        | 0.96             | invention  |
| 22   | D-II                | 0.86                                               | COMP 1           | 1%                                          | 89                       | 0.06             | comparison |
| 23   | D-II                | 0.86                                               | INV 5            | 0.5%                                        | 145                      | 0.12             | invention  |
| 24   | D-II                | 0.86                                               | COMP 2           | 1%                                          | 91                       | 0.06             | comparison |
| 25   | D-II                | 0.86                                               | INV 7            | 0.5%                                        | 151                      | 0.13             | invention  |

## EXAMPLE 4

An AgBrI tabular silver halide emulsion T-2 was prepared containing 4.05% total I distributed such that the central portion of the emulsion grains contained 1.5% I and the perimeter area contained substantially higher I, as described by Chang et al., U.S. Pat. No. 5,314,793. The emulsion grains had an average thickness of 0.13  $\mu\text{m}$  and an average circular diameter of 2.9  $\mu\text{m}$ . The emulsion was optimally chemically and spectrally sensitized by adding NaSCN, a benzothiazolium finish modifier, 0.40 mmole per mole Ag of each of the blue sensitizing dyes D-I and D-III, a substituted phenylmercaptotetrazole (PMT) antifoggant, Na<sub>3</sub>Au(S<sub>2</sub>O<sub>3</sub>)<sub>2</sub>H<sub>2</sub>O, and Na<sub>2</sub>S<sub>2</sub>O<sub>3</sub>·5H<sub>2</sub>O, and then subjecting the emulsion to a heat cycle to 65° C. The hydroxybenzene compound, 2,4-disulfocatechol (HB3) at a concentration of 1.6×10<sup>-3</sup> mole/mole Ag was added to the emulsion melt before the start of the chemical sensitization procedure. The

50

containing gelatin at 2.16 g/m<sup>2</sup>, coating surfactants, and a bisvinylsulfonylmethyl ether as a gelatin hardening agent.

For photographic evaluation, each of the coating strips was exposed for 0.02 sec to a 3000K color temperature tungsten lamp filtered to give an effective color temperature of 5500K and further filtered through a Kodak Wratten filter number 2B, and a step wedge ranging in density from 0 to 4 density units in 0.20 density steps. This exposure gives light absorbed mainly by the sensitizing dyes. In addition, a second set of coating strips was exposed for 0.02 sec to the 365 mu emission line of a Hg lamp filtered through a Kodak Wratten filter number 18A and a step wedge ranging in density from 0 to 4 density units in 0.20 density steps. This exposure gives light absorbed mainly by the silver halide material itself. The exposed film strips were developed for 3/4 minutes in Kodak C-41 color developer. S<sub>WR2B</sub>, relative sensitivity for the Kodak Wratten 2B filtered exposure, and

$S_{365}$ , relative sensitivity for the 365 nm exposure, were evaluated at a yellow density of 0.15 units above fog.

The data in Table IV show that the use of the fragmentable electron donating sensitizing agent INV 1 in this optimally sensitized, blue-dyed emulsion in color format gave significant spectral speed gains with some small fog increases. Parallel speed gains were observed for the exposures in the intrinsic silver halide region at 365 nm. The data also show that INV 1 functioned well when added during the chemical sensitization or when added after the conclusion of the chemical sensitization procedure.



TABLE IV

Speed and Fog Results for INV 1 in a fully sensitized, blue-dyed emulsion T-2, Color Format.

| Test No. | Total Amount of Inv 1 added ( $10^{-6}$ mol/mol Ag) | Position of | Photographic Sensitivity |            |           |      | Remarks    |
|----------|-----------------------------------------------------|-------------|--------------------------|------------|-----------|------|------------|
|          |                                                     |             | Addition                 | $S_{WR2B}$ | $S_{365}$ | Fog  |            |
| 1        | none                                                | —           | —                        | 100        | 100       | 0.08 | comparison |
| 2        | 3.5                                                 | after sens. | —                        | 135        | 123       | 0.08 | invention  |
| 3        | 7.0                                                 | “           | —                        | 148        | 135       | 0.10 | invention  |
| 4        | 14.0                                                | “           | —                        | 162        | 141       | 0.16 | invention  |
| 5        | 1.75                                                | in sens.    | —                        | 129        | 117       | 0.11 | invention  |
| 6        | 3.5                                                 | “           | —                        | 145        | 132       | 0.12 | invention  |
| 7        | 7.0                                                 | “           | —                        | 158        | 132       | 0.17 | invention  |

## EXAMPLE 5

The AgBrI tabular silver halide emulsion T-1 from Example 1 was optimally chemically and spectrally sensitized by adding NaSCN, 1.07 mmole per Ag mole of the blue sensitizing dye D-I,  $Na_3Au(S_2O_3)_2 \cdot 2H_2O$ ,  $Na_2S_2O_3 \cdot 5H_2O$ , and a benzothiazolium finish modifier and then subjecting the emulsion to a heat cycle to 65° C. The hydroxybenzene compound, 2,4-disulfocatechol (HB3) at a concentration of  $13 \times 10^{-3}$  mole/mole Ag and the antifogging and stabilizer tetraazaindene at a concentration of 1.75 gm/mole Ag were added to the emulsion melt after the chemical sensitization procedure. In addition, a monodisperse AgBrI tabular silver halide emulsion T-3 containing 3.6% total I was prepared according to the procedures described in Fenton et al. U.S. Pat. No. 5,476,760 in a manner such that the central portion of the emulsion grains contained essentially no I and the I was concentrated around the grain perimeter but was higher at the edges than at the corners. The emulsion grains had an average thickness of 0.12  $\mu$ m and an average circular diameter of 2.7  $\mu$ m. This emulsion T-3 was optimally chemically and spectrally sensitized by adding NaSCN, 0.77 mmole per Ag mole of the green sensitizing dye D-II, 0.17 mmole per Ag mole of the green sensitizing dye D-IV,  $Na_3Au(S_2O_3)_2 \cdot 2H_2O$ ,  $Na_2S_2O_3 \cdot 5H_2O$ , and a benzothiazolium finish modifier and then subjecting the emulsion to a heat cycle to 65° C. The hydroxybenzene compound, 2,4-disulfocatechol (HB3) at a concentration of  $13 \times 10^{-3}$  mole/mole Ag and the antifogging and stabilizer tetraazaindene at a concentration of 1.00 gm/mole Ag were added to the emulsion melt after the chemical sensitization procedure. The fragmentable electron donating sensitizing agents INV 2 and INV 5 were added to both emulsions after the additions of DSC and tetraazaindene. The variations examined are given in Table V.

The melts were prepared for coating by adding additional water, deionized gelatin, and coating surfactants. Coatings were prepared by combining the emulsion melts with a melt containing deionized gelatin and an aqueous dispersion of the cyan-forming color coupler CC-1 and coating the resulting mixture on acetate support. The final coatings contained Ag at 0.80 g/m<sup>2</sup>, coupler at 1.61 g/m<sup>2</sup>, and gelatin at 3.22 g/m<sup>2</sup>. The coatings were overcoated with a protective layer containing gelatin at 1.08 g/m<sup>2</sup>, coating surfactants, and a bisvinylsulfonylmethyl ether as a gelatin hardening agent. The coating strips obtained were then tested using the Kodak Wratten 2B exposure described in Example 4 except that the exposure time used was 0.01 s.

The data in Table V indicate that both INV 2 and INV 5 gave significant speed increases with only small fog

increases when added to the optimally sensitized, blue dyed emulsion in color format. When added to the optimally sensitized, green dyed emulsion, significantly lower concentrations of the two compounds were required to achieve a balance between speed increases and fog increases. Nevertheless, at the appropriate compound concentrations, useful speed increases in the green dyed emulsion could be obtained with only small fog increases.

total concentration of dye used, that is the sum of the amounts of conventional spectral sensitizer plus fragmentable electron donating sensitizer, was 0.91 mmole/mole Ag for coatings containing the dye D-I and 0.86 mmole/mole Ag for coatings containing the dye D-II. The sensitizing dye and fragmentable electron donating compounds were added to the emulsion at 40° C. and the coatings were prepared as described in Example 1.

D-IV



TABLE V

Speed and fog results for INV 2 and INV 5  
in fully sensitized dyed emulsions T-1 and T-3, Color Format

| Test | Type of Emulsion | Type of Sensitizing Dye | Type of FED | Amount of FED added<br>(10 <sup>-6</sup> mol/mol Ag) | Photographic Sensitivity |      |            |
|------|------------------|-------------------------|-------------|------------------------------------------------------|--------------------------|------|------------|
|      |                  |                         |             |                                                      | S <sub>WR2B</sub>        | Fog  | Remarks    |
| 1    | T-1              | D-I                     | —           | none                                                 | 100                      | 0.06 | comparison |
| 2    | T-1              | D-I                     | INV2        | 14                                                   | 132                      | 0.07 | invention  |
| 3    | T-1              | D-I                     | INV2        | 45                                                   | 135                      | 0.11 | invention  |
| 4    | T-1              | D-I                     | INV5        | 14                                                   | 135                      | 0.07 | invention  |
| 5    | T-1              | D-I                     | INV5        | 45                                                   | 126                      | 0.11 | invention  |
| 6    | T-3              | D-II + D-IV             | —           | none                                                 | 100                      | 0.09 | comparison |
| 7    | T-3              | D-II + D-IV             | INV2        | 0.45                                                 | 117                      | 0.12 | invention  |
| 8    | T-3              | D-II + D-IV             | INV2        | 1.4                                                  | 129                      | 0.33 | invention  |
| 9    | T-3              | D-II + D-IV             | INV5        | 0.45                                                 | 120                      | 0.13 | invention  |
| 10   | T-3              | D-II + D-IV             | INV5        | 1.4                                                  | 132                      | 0.38 | invention  |

## EXAMPLE 6

The sulfur sensitized emulsion T-1 as described in Example 1 used to prepare coatings containing combinations of the fragmentable electron-donating sensitizing agent INV 42 and blue spectral sensitizing dye D-I or green spectral sensitizing dye D-II. These experimental coating variations contained the hydroxybenzene 2,4-disulfocatechol (HB3) at a concentration of 13 mmole/mole Ag, added to the melt before the addition of any sensitizing dye compounds. The

For photographic evaluation, each of the coating strips was exposed for 0.1 sec to a 365 nm emission line of a Hg lamp filtered through a Kodak Wratten filter number 18A and a step wedge ranging in density from 0 to 4 density units in 0.2 density steps. The exposed film strips were developed for 6 min in Kodak Rapid X-ray Developer (KRX). S<sub>365</sub>, relative sensitivity at 365 nm, was evaluated at a density of 0.15 units above fog. For the 365 nm exposure, relative sensitivity was set equal to 100 for the control emulsion

coating (test no. 1) with no dye or fragmentable electron donating sensitizer agent added.

The data in Table VI compare the photographic sensitivities for these emulsions containing various combinations of the fragmentable electron donating sensitizer compound INV 42 with a conventional blue or green spectral sensitizing dye. The addition of conventional sensitizing dyes D-I or D-II cause some sensitivity decrease for the 365 nm exposure relative to the undyed control (tests nos. 2 and 5) due to desensitization. Improved sensitivity for the 365 nm exposure was shown for the examples which contained mixtures of D-I and a fragmentable electron donating sensitizing agent (test nos. 3,4). The data in Table VI show that Inv 42 gave a factor of 2.2 sensitivity increase relative to the comparison emulsion coating containing only D-I. A very slight increase in fog accompanied these sensitivity increases. Sensitivity increases  $S_{365}$  relative to the comparison (test no 5) of up to factor of 1.4 were also found when the fragmentable electron donating sensitizer is used in combination with a conventional green sensitizing dye (test nos. 6,7), showing that the fragmentable electron donating sensitizer is effective in ameliorating dye desensitization. However, somewhat larger increases in fog were obtained with the inventive compounds when the green sensitizing dye D-II was present.

Overall, these results show that fragmentable electron donating sensitizers Q-XY wherein X is of the general structure;



can remove dye desensitization caused by conventional sensitizing dyes, and can also give additional increases in photographic sensitivity.

TABLE VI

Speed and fog results for combinations of FED and blue or green sensitizing dye on Emulsion T-1

| Test | Type of | Total Amount of |                         | Amount of FED 42 |         | Photographic Sensitivity |      |
|------|---------|-----------------|-------------------------|------------------|---------|--------------------------|------|
|      |         | Sensitizing Dye | ( $10^{-3}$ mol/mol Ag) | FED              | Type of |                          |      |
| No.  |         |                 |                         |                  |         | $S_{365}$                | Fog  |
| 1    | none    |                 |                         | control          | 0       | 100                      | 0.04 |
| 2    | D-I     |                 | 0.91                    | none             | 0       | 80                       | 0.04 |
| 3    | D-I     |                 | 0.91                    | INV 42           | 1%      | 162                      | 0.06 |
| 4    | D-I     |                 | 0.91                    | INV 42           | 1%      | 174                      | 0.09 |
| 5    | D-II    |                 | 0.86                    | none             | 0       | 83                       | 0.08 |
| 6    | D-II    |                 | 0.86                    | INV 42           | 0.031%  | 97                       | 0.08 |
| 7    | D-II    |                 | 0.86                    | INV 42           | 0.1%    | 115                      | 0.13 |

The invention has been described in detail with particular reference to preferred embodiments, but it will be understood that variations and modifications can be effected within the spirit and scope of the invention.

What is claimed is:

1. A photographic element comprising a support and at least one silver halide emulsion layer in which the silver halide is sensitized with a compound of the formula:

wherein Q represents the atoms necessary to form a chromophore comprising an amidinium-ion, a carboxyl-ion or dipolar-amidic chromophoric system when conjugated with XY, and XY is a fragmentable electron donor moiety in which X is an electron donor group and Y is a leaving group other than hydrogen, and wherein:

1) XY has an oxidation potential between 0 and about 1.4 V;

2) the oxidized form of XY undergoes a bond cleavage reaction to give the radical  $X^{\cdot}$  and the leaving fragment Y.

2. A photographic element comprising a support and at least one silver halide emulsion layer in which the silver halide is sensitized with a compound of the formula:

wherein Q represents the atoms necessary to form a chromophore comprising an amidinium-ion, a carboxyl-ion or dipolar-amidic chromophoric system when conjugated with XY, and XY is a fragmentable electron donor moiety in which X is an electron donor group and Y is a leaving group other than hydrogen, and wherein:

1) XY has an oxidation potential between 0 and about 1.4 V;

2) the oxidized form of XY undergoes a bond cleavage reaction to give the radical  $X^{\cdot}$  and the leaving fragment Y; and

3) the radical  $X^{\cdot}$  has an oxidation potential  $<-0.7V$ .

3. A photographic element according to claim 1 or claim 2, wherein Q is represented by the general formula:





85

-continued



86

-continued



and



25 8. A photographic element according to claim 1 or claim 2, wherein Q is of the formula:



35 wherein:

X<sub>2</sub> is O, S, N, or C(R<sub>52</sub>)<sub>2</sub>, where R<sub>52</sub> is substituted or unsubstituted alkyl,  
each R<sub>50</sub> is independently a hydrogen atom, a halogen atom, a substituted or unsubstituted alkyl group, or substituted or unsubstituted aryl group;  
a is an integer of 1-4; and  
R<sub>51</sub> is substituted or unsubstituted alkyl, or substituted or unsubstituted aryl.

40 9. A photographic element according to claim 1 or claim 2, wherein X is of formula (I)



55 wherein:

m: 0, 1;  
Z: O, S, Se, Te;  
Ar: aryl group; or heterocyclic group;  
R<sub>1</sub>: R, carboxyl, amide, sulfonamide, halogen, NR<sub>2</sub>, (OH)<sub>n</sub>, (OR<sup>1</sup>)<sub>n</sub> or (SR)<sub>n</sub> where R<sup>1</sup> is alkyl or substituted alkyl;  
n: 1-3;  
R<sub>2</sub>: R, Ar';  
R<sub>3</sub>: R, Ar';  
60 R<sub>2</sub> and R<sub>3</sub> together can form 5- to 8-membered ring;  
R<sub>2</sub> and Ar: can be linked to form 5- to 8-membered ring;

87

R3 and Ar: can be linked to form 5- to 8-membered ring;  
 Ar': aryl group or heterocyclic group; and  
 R: a hydrogen atom or an unsubstituted or substituted alkyl group.

10. A photographic element according to claim 9 wherein X is selected from the group consisting of:



wherein R is a hydrogen atom or a substituted or unsubstituted alkyl group.

88

11. A photographic element according to claim 1 or claim 2, wherein X is of formula (II)



wherein:

Ar: aryl group; or heterocyclic group;

R<sub>4</sub>: a substituent having a Hammett sigma value of -1 to +1, preferably -0.7 to +0.7;

R<sub>5</sub>: R, Ar'

R<sub>6</sub> and R<sub>7</sub>: R, Ar'

R<sub>5</sub> and Ar: can be linked to form 5- to 8-membered ring;

R<sub>6</sub> and Ar: can be linked to form 5- to 8-membered ring (in which case, R<sub>6</sub> can be a hetero atom);

R<sub>5</sub> and R<sub>6</sub>: can be linked to form 5- to 8-membered ring;

R<sub>6</sub> and R<sub>7</sub>: can be linked to form 5- to 8-membered ring;

Ar': aryl group or a heterocyclic group; and

R: hydrogen atom or an unsubstituted or substituted alkyl group.

12. A photographic element according to claim 11, wherein X is selected from the group consisting of:



wherein R<sub>11</sub> and R<sub>12</sub> are independently H, alkyl, alkoxy, alkylthio, halo, carbamoyl, amido, formyl, sulfonyl, sulfonamido or nitrile and R is a hydrogen atom or an unsubstituted or substituted alkyl group.

13. A photographic element according to claim 11, wherein X is selected from the group consisting of

89



wherein  $Z_1$  is covalent bond, S, O, Se, NR, CR<sub>2</sub>, CR=CR or CH<sub>2</sub>CH<sub>2</sub> and R is a hydrogen atom or a substituted or unsubstituted allyl group.

14. A photographic element according to claim 11, wherein X has the structure:



wherein  $Z_2$  is S, O, Se, NR, CR<sub>2</sub> or CR=CR, and R<sub>13</sub> is an unsubstituted or substituted alkyl or aryl group, and R<sub>14</sub> is a hydrogen atom or an unsubstituted or substituted alkyl or aryl group and R is a hydrogen atom or a substituted or unsubstituted alkyl group.

**15. A photographic element according to claim 1 or claim 2, wherein X is of formula (III)**



wherein:

W=O, S, Se;

Ar: aryl group; or heterocyclic group;

R<sub>2</sub>: R, carboxyl, NR<sub>2</sub>, (OR)<sub>n</sub>, or (SR)<sub>n</sub> (n=1-3);

R<sub>g</sub>, R, carboxyl, NH

Ar': aryl group or heterocyclic group;

Ar: aryl group or heterocyclic group;  
 $R_9$  and Ar: can be linked to form 5- to 8-membered ring;  
 and

R: a hydrogen atom or an unsubstituted or substituted alkyl group

90

16. A photographic element according to claim 15, wherein X is selected from the group consisting of:



wherein n is 1-3, and R is a hydrogen atom or an unsubstituted or substituted alkyl group.

17. A photographic element according to claim 1 or claim  
30 2, wherein X is of formula (IV):



wherein "ring" represents a substituted or unsubstituted 5-, 40 6- or 7-membered unsaturated ring.

**18.** A photographic element according to claim 17, wherein X is selected from the group consisting of:



wherein:

$Z_3$  is O, S, Se or NR;

$R_{12}$  is QR or NR<sub>12</sub> and

60  $R_{15}$  is OR or  $NH_2$ , and  
 $R_{16}$  unsubstituted alkyl or substituted alkyl and R is a hydrogen atom or an unsubstituted or substituted alkyl group.

19. A photographic element according to claim 1 or claim 2, wherein Y is:

65 (1) X', where X' is an X group as defined in structures I-IV and may be the same as or different from the X group to which it is attached



**20.** A photographic element according to claim **19**, wherein  $\text{Y}$  is  $\text{COO}^-$ ,  $\text{Si}(\text{R}')_3$  or  $\text{X}'$ .

**21.** A photographic element according to claim **20**, wherein  $\text{Y}$  is  $\text{COO}^-$  or  $\text{Si}(\text{R}')_3$ .

**22.** A photographic element according to claim **1** or claim **2**, wherein  $\text{Q-XY}$  is a compound of the formula



-continued



**23.** A photographic element according to claim **1** or claim **2**, wherein  $\text{Q-XY}$  is a compound of the formula



**93**

-continued

**94**

-continued



or

15  
20

25

30  
3540  
4550  
55

60



**24.** A photographic element according to claim 1 or claim 2, wherein Q-XY is a compound of the formula



**26.** A photographic element according to claim 1 or claim 2, wherein Q-XY is a compound of the formula



99



100

27. A photographic element according to claim 1 or claim 2, wherein Q-XY is a compound of the formula

$W_2$  is a counterion as necessary to balance the charge;



wherein  $E_1$ ,  $D_1$ ,  $J$ ,  $p$ ,  $q$  and  $W_2$  are as defined above for formula (XII) and  $G$  represents

**28.** A photographic element according to claim 1 or claim 2, wherein the emulsion layer further contains a sensitizing dye.

29. A photographic element according to claim 28, wherein the sensitizing dye is selected from dyes of formula (XII) through (XVI):



35 wherein  $E_2$  represents the atoms necessary to complete a substituted or unsubstituted heterocyclic nucleus, and  $F$  and  $F'$  each independently represents a cyano radical, an ester radical, an acyl radical, a carbamoyl radical or an alkylsul-  
40 fonyl radical;

wherein:

$E_1$  and  $E_4$  represent the atoms necessary to form a 45 substituted or unsubstituted hetero ring and may be the same or different

each J independently represents a substituted or unsubstituted methine group,

q is a positive integer of from 1 to 4,

p and r each independently represents 0 or

D<sub>1</sub> and D<sub>2</sub> each independently represents sub-

unsubstituted alkyl or unsubstituted aryl, and



wherein  $D_1$ ,  $E_1$ ,  $J$ ,  $p$ ,  $q$  and  $W_2$  are as defined above for formula (XII), and  $G_2$  represents a substituted or unsubstituted amino radical or a substituted or unsubstituted aryl radical:



**101**

wherein  $D_1$ ,  $E_1$ ,  $D_2$ ,  $E_4$ ,  $J$ ,  $p$ ,  $q$ ,  $r$  and  $W_2$  are as defined for formula (XII) above, and  $E_3$  is defined the same as  $E_2$  for formula (XIII) above;



5

10

15

wherein  $D_1$ ,  $E_1$ ,  $J$ ,  $G$ ,  $p$ ,  $q$ ,  $r$  and  $W_2$  are as defined above for formula (XII) above and  $E_3$  is as defined for formula (XIII) above.

**30.** A photographic element according to claim 1 or claim 2, comprising a plurality of layers wherein one or more of the layers of the element contains a hydroxybenzene compound.

**31.** A photographic element according to claim 30, wherein the hydroxybenzene compound has the formula:

**102**

wherein  $V$  and  $V'$  each independently represent  $—H$ ,  $—OH$ , a halogen atom,  $—OM$  (where  $M$  is alkali metal ion), an alkyl group, a phenyl group, an amino group, a carbonyl group, a sulfone group, a sulfonated phenyl group, a sulfonated alkyl group, a sulfonated amino group, a carboxyphenyl group, a carboxyalkyl group, a carboxyamino group, a hydroxyphenyl group, a hydroxyalkyl group, an alkylether group, an alkylphenyl group, an alkylthioether group, or a phenylthioether group.

\* \* \* \* \*